# EUROPEAN PATENT SPECIFICATION

(11) **EP 3 522 178 B1**
(45) Date of publication and mention of the grant of the patent: **23.02.2022**
(21) Application number: 18215888.1
(22) Date of filing: 24.12.2018
(51) Int. Cl.: H01F 1/057, H01F 41/02

(54) **RARE EARTH MAGNET AND PRODUCTION METHOD THEREOF**
SELTENERDMAGNET UND HERSTELLUNGSVERFAHREN DAFÜR
AIMANT DE TERRES RARES ET PROCÉDÉ DE PRODUCTION ASSOCIÉ

(30) Priority: 28.12.2017 JP 2017254475; 10.08.2018 JP 2018151433; 27.11.2018 JP 2018221584
(43) Date of publication of application: 07.08.2019
(73) Proprietor: TOYOTA JIDOSHA KABUSHIKI KAISHA, Toyota-shi, Aichi-ken, 471-8571 (JP)
(72) Inventor: Ito, Masaaki, Aichi-ken, Aichi 471-8571 (JP); Shoji, Tetsuya, Aichi-ken, Aichi 471-8571 (JP); Sakuma, Noritsugu, Aichi-ken, Aichi 471-8571 (JP); Ichigozaki, Daisuke, Aichi-ken, Aichi 471-8571 (JP)
(74) Representative: J A Kemp LLP

(56) References cited:
- JP-A- 2016 111 136
- US-A- 5 129 963
- US-A- 6 136 099
- US-A1- 2016 141 083

## Description

### [TECHNICAL FIELD]

The present disclosure relates to an R-Fe-B-based rare earth magnet, wherein R is a rare earth element, and a production method thereof. More specifically, the present disclosure relates to an R-Fe-B-based rare earth magnet protected from reduction in the coercive force at high temperatures, and a production method thereof.

### [BACKGROUND ART]

An R-Fe-B-based rare earth magnet has a main phase and a grain boundary phase present around the main phase. The main phase has a composition represented by R₂Fe₁₄B and is a magnetic phase. Due to this main phase, strong magnetism is exhibited. On the other hand, the grain boundary phase is present around the main phase and magnetically isolates the main phases from one another. The coercive force of the R-Fe-B-based rare earth magnet is enhanced by this magnetic isolation.

In order to enhance the magnetic isolation effect, various attempts are being made. For example, Patent Document 1 discloses a rare earth magnet using, as a precursor, a rare earth magnet having a main phase and a grain boundary phase, in which a modifier is infiltrated into the inside of the precursor.

In the rare earth magnet disclosed in Patent Document 1, the coercive force of the entire rare earth magnet is enhanced by having an intermediate phase between the main phase and the grain boundary phase.

### [RELATED ART]

### [Patent Document]

[Patent Document 1] International Publication No. 2014/196605A1

US 6 136 099 A discloses a rare earth-iron series magnet formed from an alloy ingot using a one-step hot working process. The alloy ingot includes between about 8 and 30 atomic percent of at least one rare earth element, between about 2 and 28 atomic percent of boron, less than about 50 atomic percent of cobalt, less than about 15 atomic percent of aluminum and the balance of iron and other impurities that are inevitably included during the preparation process. The alloy is cast to obtain a cast ingot and the hot working is performed on the cast ingot at a temperature of greater than about 500 DEG C. in order to make the crystal grains of the ingot fine and to align the axis of the grains in a desired direction.

JP 2016 111136 A discloses a rare-earth magnet excellent in high temperature coercive force, while reducing the amount of Nd. A crystal grain having a whole composition of (CeNd)FeCoBM (in the formula, M is at least one kind of Ga, Al, Cu, Au, Ag, Zn, In, Mn, 0≤x≤0.75, 5≤y≤20, 4≤z≤6.5, 0≤w≤8, 0≤v≤2) is constituted of a core and a shell therearound. The Nd concentration is higher in the shell than in the core.

### [SUMMARY OF THE INVENTION]

### [Problems to be Solved by the Invention]

The R-Fe-B-based rare earth magnet is of high performance, and therefore its use is expanding to a variety of fields. Consequently, the opportunity of using the R-Fe-B-based rare earth magnet under a high-temperature environment is increased. In addition, when the R-Fe-B-based rare earth magnet is used in a high-power motor and high output was maintained for a long time, the R-Fe-B-based rare earth magnet is sometimes subjected to high temperatures due to self-heating of the motor.

It is known that when the R-Fe-B-based rare earth magnet is subjected to high temperatures, the coercive force may decrease.

Accordingly, the present inventors have found a problem that an R-Fe-B-based rare earth magnet protected from reduction in the coercive force even at high temperatures is demanded. Incidentally, in the present description, the high temperature indicates a range from 130 to 170°C, particularly from 140 to 160°C, the room temperature indicates a range from 20 to 25°C, and the R-Fe-B-based rare earth magnet indicates a magnet having a main phase and a grain boundary phase present around the main phase, the main phase containing a phase having a composition represented by R₂Fe₁₄B.

The present disclosure have been made to solve the problem above. An object of the present disclosure is to provide an R-Fe-B-based rare earth magnet protected from reduction in the coercive force even at high temperatures and a production method thereof.

### [Means to Solve the Problems]

As a result of many intensive studies to attain the object above, the present inventors have accomplished the rare earth magnet of the present disclosure and the production method thereof. The rare earth magnet of the present disclosure and the production method thereof include the following embodiments.
<1> A rare earth magnet including:
   a main phase, and
   a grain boundary phase present around the main phase,
      wherein the overall composition is represented by the formula,
      wherein Ndₓ(Ce, La)_{(1-x-y)}R¹y)ₚFe_{(100-p-q-r-s)}Co_{q}BᵣM¹ₛ· (R²_{z}R³_{w}M²_{1-z-w})ₜ,
      wherein R¹ is one or more members selected from rare earth elements other than Nd, Ce and La, R² is one or more members selected from Pr, Nd, Pm, Sm, Eu and Gd, R³ is one or more members selected from rare earth elements other than R², M¹ represents one or more members selected from Ga, Al, Cu, Au, Ag, Zn, In and Mn, and an unavoidable impurity element, M² represents an alloy element for decreasing the melting point of R²_{z}R³_{w}M²_{1-z-w} to be lower than the melting point of R² by alloying with R² and R³, and an unavoidable impurity element,
      wherein p, q, r, s, and t are, in at%,
         5.0≤p≤20.0,
         0≤q≤8.0,
         4.0≤r≤6.5,
         0≤s≤2.0, and
         0≤t≤10.0, and
      wherein x, y, z, and w are, by molar ratio,
         0.4≤x≤0.8,
         0≤y≤0.1,
         0.5≤z≤0.8, and
         0≤w≤0.1, and
      wherein La is contained in an amount of 1/9 to 3 times by molar ratio relative to Ce, characterized in that an average grain size of the main phase is from 1 to 1,000 nm, wherein the average grain size of the main phase is calculated in accordance with the method defined in the description.
<2> The rare earth magnet according to item <1>, wherein La is contained in an amount of 1/9 to 2 times by molar ratio relative to Ce.
<3> The rare earth magnet according to item <1> or <2>,
   wherein: an intermediate phase is further provided between the main phase and the grain boundary phase,
   wherein t is 0.1≤t≤10.0, and
   wherein the concentration of R² is higher in the intermediate phase than in the main phase.
<4> The rare earth magnet according to any one of items <1> to <3>, wherein R² is Nd.
<5> The rare earth magnet according to item <3> or <4>, wherein the concentration of R² is higher by 1.5 to 8.0 times in the intermediate phase than in the main phase.
<6> The rare earth magnet according to any one of items <3> to <5>, wherein the thickness of the intermediate phase is from 2 to 100 nm.
<7> A method for producing a rare earth magnet, including:
   preparing a molten metal having a composition represented by the formula: Ndₓ(Ce, La)_{(1-x-y)}R¹_{y})ₚFe_{(100-p-q-r-s)}Co_{q}BᵣM¹ₛ,
      wherein R¹ is one or more members selected from rare earth elements other than Nd, Ce and La, M¹ represents one or more members selected from Ga, Al, Cu, Au, Ag, Zn, In and Mn, and an unavoidable impurity element,
      wherein p, q, r, and s are, in at%,
         5.0≤p≤20.0,
         0≤q≤8.0,
         4.0≤r≤6.5, and
         0≤s≤2.0, and
      wherein x and y are, by molar ratio,
         0.4≤x≤0.8,and
         0≤y≤0.1, and
      wherein La is contained in an amount of 1/9 to 3 times by molar ratio relative to Ce,
   quenching the molten metal to obtain a ribbon,
   compressing a plurality of ribbons by hot working to obtain a molded body, and
   compressing the molded body by hot working to obtain a compressed body, wherein an average grain size of the main phase (10) is from 1 to 1000 nm, wherein the average grain size of the main phase (10) is calculated in accordance with the method defined in the description.
<8> The method according to item <7>, wherein the molten metal contains La in an amount of 1/9 to 2 times by molar ratio relative to Ce.
<9> The method according to item <7> or <8>, including:
   preparing a modifier containing an alloy represented by the formula: R²_{z}R³_{w}M²_{1-z-w},
      wherein R² is one or more members selected from Pr, Nd, Pm, Sm, Eu and Gd, R³ is one or more members selected from rare earth elements other than R², M² represents an alloy element for decreasing the melting point of R²_{z}R³_{w}M²_{1-z-w} to be lower than the melting point of R² by alloying with R² and R³, and an unavoidable impurity element,
      wherein z and w are, by molar ratio, 0.5≤z≤0.8 and 0≤w≤0.1,
   contacting the compressed body and the modifier with each other to obtain a contact body, and
   heat-treating the contact body to infiltrate a melt of the modifier into the inside of the compressed body.
<10> The method according to item <9>, wherein R² is Nd.
<11> The method according to any one of items <7> to <10>, wherein the molded body is compressed at a strain rate of 0.001/s or more and less than 0.1/s, a reduction ratio of 50 to 70%, and a temperature of 700 to 800°C to obtain a compressed body.

### [Effects of the Invention]

According to the present disclosure, a rare earth magnet protected from reduction in the coercive force at high temperatures by causing Nd, Ce and La to be present together and setting the content ratio between Ce and La to a predetermined range, and a production method thereof can be provided.

### [BRIEF DESCRIPTION OF THE DRAWINGS]

[Fig. 1] Fig. 1 is a diagram illustrating the content ratio of Nd, Ce and La.
[Fig. 2] Fig. 2 is a diagram schematically illustrating one embodiment of the texture of the rare earth magnet according to the present disclosure.
[Fig. 3] Fig. 3 is a diagram illustrating another embodiment of the texture of the rare earth magnet according to the present disclosure.
[Fig. 4] Fig. 4 is a graph illustrating the relationship between the temperature and the cohesive force with respect to the samples of Example 15 and Comparative Example 1.
[Fig. 5] Fig. 5 is a diagram illustrating the relationship between the temperature and the residual magnetization with respect to the samples of Example 15 and Comparative Example 1.
[Fig. 6] Fig. 6 is a diagram illustrating the positions for texture observation and component analysis with respect to the sample of Example 6.
[Fig. 7] Fig. 7 is a diagram illustrating the results of texture observation and composition analysis with respect to the sample of Example 6 (first visual field).
[Fig. 8] Fig. 8 is a diagram illustrating the results of texture observation and composition analysis with respect to the sample of Example 6 (second visual field).
[Fig. 9] Fig. 9 is a diagram illustrating the positions for texture observation and composition analysis with respect to the sample of Example 12.
[Fig. 10] Fig. 10 is a diagram illustrating the results of texture observation and composition analysis with respect to the sample of Example 12 (first visual field).
[Fig. 11] Fig. 11 is a diagram illustrating the results of texture observation and composition analysis with respect to the sample of Example 12 (second visual field).
[Fig. 12] Fig. 12 is a diagram illustrating the positions for texture observation and composition analysis with respect to the sample of Example 17.
[Fig. 13] Fig. 13 is a diagram illustrating the results of texture observation and composition analysis with respect to the sample of Example 17 (first visual field).
[Fig. 14] Fig. 14 is a diagram illustrating the results of texture observation and composition analysis with respect to the sample of Example 17 (second visual field).
[Fig. 15] Fig. 15 is a diagram illustrating one example of the grain size t of a crystal grain with respect to the sample of Example 39.
[Fig. 16] Fig. 16 is a diagram illustrating one example of the grain size t of a crystal grain with respect to the sample of Example 40.
[Fig. 17] Fig. 17 is a diagram illustrating one example of the grain size t of a crystal grain with respect to the sample of Example 6.
[Fig. 18] Fig. 18 is a diagram illustrating one example of the grain size t of a crystal grain with respect to the sample of Example 12.
[Fig. 19] Fig. 19 is a diagram illustrating the results of texture observation and the positions for composition analysis with respect to the sample of Example 39.
[Fig. 20] Fig. 20 is a diagram illustrating the results of composition analysis at a position indicated by a white line in Fig. 19.
[Fig. 21] Fig. 21 is a diagram illustrating the results of texture observation and the positions for composition analysis with respect to the sample of Example 40.
[Fig. 22] Fig. 22 is a diagram illustrating the results of composition analysis at a position indicated by a white line in Fig. 21.
[Fig. 23] Fig. 23 is a diagram illustrating the results of texture observation and the positions for composition analysis with respect to the sample of Example 6.
[Fig. 24] Fig. 24 is a diagram illustrating the results of composition analysis at a position indicated by a white line in Fig. 23.
[Fig. 25] Fig. 25 is a diagram illustrating the results of texture observation and the positions for composition analysis with respect to the sample of Example 12.
[Fig. 26] Fig. 26 is a diagram illustrating the results of composition analysis at a position indicated by a white line in Fig. 25.

### [Mode for Carrying Out the Invention]

The embodiments of the rare earth magnet according to the present disclosure and the production method thereof are described in detail below. Incidentally, the embodiments set forth below should not be construed to limit the rare earth magnet according to the present disclosure and the production method thereof, as long as remaining within the scope of the appended claims.

In the R-Fe-B-based rare earth magnet, when 1) the grain size of the main phase is reduced, 2) the anisotropic magnetic field of the main phase is increased, and 3) main phases are magnetically isolated from one another, the coercive force is enhanced.

In order to reduce the grain size of the main phase, in the R-Fe-B-based rare earth magnet, the main phase is nanocrystallized. Consequently, in the R-Fe-B-based rare earth magnet, a large amount of R₂Fe₁₄B phase is present as the main phase, and a grain boundary phase is present around the main phase. In the grain boundary phase, an R-rich phase containing excess R, and a small amount of magnetic phase containing Fe (for example, RFe₂ phase) are present.

In the Nd₂Fe₁₄B phase, the anisotropic magnetic field at room temperature is high, but the Curie point is 320°C and is not so high. Accordingly, even if the Curie point is not reached, at high temperatures, the anisotropic magnetic field of the Nd₂Fe₁₄B phase is reduced. On the other hand, the Fe-containing magnetic phase (for example, RFe₂ phase) is paramagnetic at a temperature higher than the normal temperature but has a possibility of propagating the interaction of magnetic spins between Nd₂Fe₁₄B phases (between crystal grains). When a large amount of Nd₂Fe₁₄B phase is present as the main phase, the coercive force is high at room temperature, because the Fe-containing magnetic phase in the grain boundary phase has a small effect. However, at high temperature, the Fe-containing magnetic phase in the grain boundary phase has the effect of propagating the interaction of magnetic spins between Nd₂Fe₁₄B phases (between crystal grains), and the grain size of the main phase is thereby apparently increased, presenting the possibility of reducing the effect of nanocrystallization of the main phase. As a result, the coercive force rapidly decreases.

When R of the R-Fe-B-based rare earth magnet contains Nd, Ce and La, the anisotropic magnetic field of (Nd, Ce, La)₂Fe₁₄B is lower than the anisotropic magnetic field of Nd₂Fe₁₄B at both room temperature and high temperature. Hereinafter, the R-Fe-B-based rare earth magnet containing Nd, Ce and La is sometimes referred to as "(Nd, Ce, La)-Fe-B-based rare earth magnet".

Although not bound by theory, in the (Nd, Ce, La)-Fe-B-based rare earth magnet, when the content ratio between Ce and La is in a predetermined range, the stability of the Fe-containing magnetic phase (e.g., RFe₂ phase) in the grain boundary phase decreases, compared with the Nd-Fe-B-based rare earth magnet. Consequently, in the (Nd, Ce, La)-Fe-B-based rare earth magnet, Fe in the grain boundary phase is likely to contribute to the production of a phase other than the Fe-containing magnetic phase. The phase other than the Fe-containing magnetic phase includes CeFe₂ phase, etc.

Formation of the (Nd, Ce, La)₂Fe₁₄B phase brings about an increase in the total number of main phases, and consequent replacement of Nd by Ce and La compensates for the reduction in the anisotropic magnetic field and suppresses the reduction in the coercive force of the entire (Nd, Ce, La)-Fe-B-based rare earth magnet. This enhancement of coercive force is prominent at high temperatures. Incidentally, in the present description, although not bound by theory, with respect to the (Nd, Ce, La)₂Fe₁₄B phase, Ce or La is present at the position of Nd of the Nd₂Fe₁₄B phase.

In addition, when the (Nd, Ce, La)-Fe-B-based rare earth magnet is used as a precursor and a modifier containing R² is infiltrated into the inside of the precursor, depending on the infiltration amount of the alloy from the modifier, an intermediate phase is formed between the main phase and the grain boundary phase.

Although not bound by theory, it is considered that part of Ce and/or La present in the main phase of the precursor is replaced by R² and an intermediate phase is thereby formed. Accordingly, in the intermediate phase, the concentration of R² is higher than in the main phase of the precursor and in turn, the anisotropic magnetic field of the intermediate phase is higher than the anisotropic magnetic field of the main phase of the precursor. At high temperature, the anisotropic magnetic field of the intermediate phase is reduced. However, even at high temperature, the anisotropic magnetic field of the intermediate phase is higher than the anisotropic magnetic field of the main phase of the precursor by the amount corresponding to the R² concentration that is increased compared with the main phase of the precursor. This contributes to the protection from reduction in the coercive force.

From the matters described hereinbefore, the present inventors have found that with respect to the R-Fe-B-based rare earth magnet, the reduction in the coercive force at high temperatures can be suppressed.

The configuration requirements of the rare earth magnet according to the present disclosure and the production method thereof, based on the finding above, are described below.

### <<Rare Earth Magnet>>

First, the configuration requirements of the rare earth magnet of the present disclosure are described.

### <Overall Composition>

The overall composition of the rare earth magnet of the present invention is represented by the formula: (Ndₓ(Ce, La)_{(1-x-y)}R¹_{y})ₚFe_{(100-p-q-r-s)}Co_{q}BᵣM¹s·(R²_{z}R³_{w}M²_{1-z-w})_{t.}

In the formula above, (R²_{z}R³_{w}M²_{1-z-w})ₜ represents a composition derived from the later-described modifier. In the case of not infiltrating a modifier, t=0, and the overall composition of the rare earth magnet of the present disclosure is represented by (Ndₓ(Ce, La)_{(1-x-y)}R¹_{y})ₚFe_{(100-p-q-r-s)}Co_{q}BᵣM¹ₛ.

On the other hand, in the case of infiltrating a modifier, t is a positive value and is not 0, and (Ndₓ(Ce, La)_{(1-x-y)}R¹_{y})ₚFe_{(100-p-q-r-s)}Co_{q}BᵣM¹ₛ represents a composition of the rare earth magnet precursor.

In the formula above, Nd stands for neodymium, Ce stands for cerium, La stands for lanthanum, R¹ is one or more members selected from rare earth elements other than Nd, Ce and La, Fe stands for iron, Co stands for cobalt, and B stands for boron. M¹ represents one or more members selected from Ga, Al, Cu, Au, Ag, Zn, In and Mn, and an unavoidable impurity element. Ga stands for gallium, Al stands for aluminum, Cu stands for copper, Au stands for gold, Ag stands for silver, Zn stands for zinc, In stands for indium, and Mn stands for manganese. R² is one or more members selected from Pr, Nd, Pm, Sm, Eu and Gd. Pr stands for praseodymium, Nd stands for neodymium, Pm stands for promethium, Sm stands for samarium, Eu stands for europium, and Gd stands for gadolinium. M² represents an alloy element for decreasing the melting point of R²_{z}R³_{w}M²_{1-z-w} to be lower than the melting point of R² by alloying with R² and R³, and an unavoidable impurity element.

In the present description, the rare earth element includes 17 elements of Sc, Y, La, Ce, Pr, Nd, Pm, Sm, Eu, Gd, Tb, Dy, Ho, Er, Tm, Yb, and Lu. Of these, Sc, Y, La, and Ce are a light rare earth element, Pr, Nd, Pm, Sm, Eu, and Gd are a medium rare earth element, and Tb, Dy, Ho, Er, Tm, Yb, and Lu are a heavy rare earth element. Incidentally, in general, the rarity of the heavy rare earth element is high, and the rarity of the light rare earth element is low. The rarity of the medium rare earth element is between the heavy rare earth element and the light rare earth element.

Next, p, q, r, s and t, and x, y, z and w are described. In the following description, the case of infiltrating a modifier is explained. As for the case of not infiltrating a modifier, the "rare earth magnet precursor" is read as "rare earth magnet", and the description of items derived from a modifier is treated as non-existing.

In the rare earth magnet precursor, p is the total content of Nd, Ce, La and R¹, q is the content of Co, r is the content of B (boron), and s is the content of M¹. With respect to the items derived from a modifier, t is the infiltration amount of an alloy from the modifier, relative to the rare earth magnet precursor, and is the total content of R², R³ and M². Each of the values of p, q, r, s and t is at%.

In the rare earth magnet precursor, each of the values of x and y is the following content ratio (molar ratio). x represents the content ratio of Nd relative to the total content of Nd, Ce, La and R¹, and y represents the content ratio of R¹ relative to the total content of Nd, Ce, La and R¹ . With respect to the items derived from a modifier, each of the values of z and w is the following content ratio (molar ratio). z is the content ratio of R² relative to the total content of R², R³ and M², and w represents the content ratio of R³ relative to the total content of R², R³ and M².

The constituent elements of the rare earth magnet precursor represented by the formula above are described below.

### <Nd>

Nd is an element essential for the rare earth magnet precursor of the present disclosure. By containing Nd, high magnetization can be exhibited at room temperature and high temperature. In addition, at room temperature, the Nd₂Fe₁₄B phase has a high anisotropic magnetic field.

### <Ce>

Ce is an element essential for the rare earth magnet precursor of the present disclosure. When Nd in the main phase (Nd₂Fe₁₄B phase) is replaced by Ce, an Fe-containing magnetic phase, i.e., a CeFe₂ phase, in the grain boundary phase is readily formed. The CeFe₂ phase is paramagnetic and is expected to have an effect of propagating the interaction of magnetic spins between main phases to reduce the coercive force. In order to suppress the reduction in the coercive force, it is necessary to reduce the stability of the Fe-containing magnetic phase in the grain boundary phase.

In addition, Ce can have an atomic valence of trivalence or tetravalence. Although not bound by theory, a lot of Ce becomes trivalent due to an action of La. In the trivalent Ce, 4f electrons are localized, and therefore magnetization is advantageously enhanced.

### <La>

La is an element essential for the rare earth magnet precursor of the present disclosure. Nd in the main phase (Nd₂Fe₁₄B phase) is replaced by La, and the stability of the Fe-containing magnetic phase in the grain boundary phase is reduced, because compounds of a transition metal such as La and Fe are thermodynamically unstable as a whole and are not mixed with one another. That is, the addition of La is expected to provide an effect of forming an RFe₂ phase. Accordingly, La greatly contributes to protection from reduction in the coercive force. Moreover, La is advantageously inexpensive compared with Nd. In addition, when Ce is added, a CeFe₂ phase is likely to be formed, and the coercive force is reduced. However, when La is added together with Ce, the formation of CeFe₂ phase is suppressed, and the propagation of interaction of magnetic spins between grains in the main phase is restricted.

### <Content Ratio of Nd, Ce and La>

As described above, x is the content ratio of Nd. The saturation magnetization and anisotropic magnetic field are higher in the Nd₂Fe₁₄B phase than in Ce₂Fe₁₄B phase and La₂Fe₁₄B phase. Accordingly, when x is 0.40 or more, desired magnetization and coercive force are readily obtained in the rare earth magnet of the present disclosure. From this viewpoint, x may be 0.45 or more, 0.50 or more, or 0.55 or more. On the other hand, when x is 0.80 or less, it is unlikely that the content ratio of Ce and La is too small and the actions and effects of Ce and La are hardly obtained. From this viewpoint, x may be 0.75 or less, 0.70 or less, or 0.65 or less.

In the rare earth magnet precursor, the content of La is, by molar ratio, from 1/9 to 3 times relative to the content of Ce. Fig. 1 is a diagram illustrating the content ratio of Nd, Ce and La. In Fig. 1, the straight line denoted by (1) indicates a composition in which the content of La is, by molar ratio, 1/9 times relative to the content of Ce; the straight line denoted by (2) indicates a composition in which the content of La is, by molar ratio, 1/3 times relative to the content of Ce; the straight line denoted by (3) indicates a composition in which the content of La is, by molar ratio, 2/3 times relative to the content of Ce; and the straight line denoted by (4) indicates a composition in which the content of La is, by molar ratio, 3 times relative to the content of Ce.

More specifically, these are rephrased as follows. The straight line of (1) indicates a composition at Ce:La=1:1/9; the straight line of (2) indicates a composition at Ce:La=1:1/3; the straight line of (3) indicates a composition at Ce:La=1:2/3; and the straight line of (4) indicates a composition at Ce:La=1:3.

As described above, the content ratio x of Nd is from 0.4 to 0.8, and therefore in Fig. 1, the composition of the rare earth magnet precursor of the present disclosure is denoted by a portion in which the region sandwiched by "Nd80" and "Nd40" and the region sandwiched by straight line (1) and straight line (4) are overlapped.

When the content of La is, by molar ratio, 1/9 times or more relative to the content of Ce, desired magnetization can be obtained at room temperature and high temperature. From this viewpoint, the content is preferably 1/8 times or more, more preferably 1/7 times or more. On the other hand, when the content of La is by molar ratio, 3 times or less relative to the content of Ce, Nd of the grain boundary phase is replaced by Ce and/or La, thereby reducing the stability of the Fe-containing magnetic phase (e.g., RFe₂ phase), and the content (volume ratio) of the Fe-containing magnetic phase decreases. As a result, the grain boundary phase restricts the effect of propagating the interaction of magnetic spins between main phases and suppresses the reduction in the coercive force at high temperature. From this viewpoint, the content is preferably 5/2 times or less, more preferably 2 times or less.

### <R¹>

R¹ is one or more members selected from rare earth elements other than Nd, Ce and La. The rare earth magnet of the present disclosure contains Nd, Ce and La as essential components. It is difficult for raw materials of these essential components not to contain the rare earth element R¹ other than Nd, Ce and La at all. However, when the value of the content ratio y of R¹ is from 0 to 0.1, the properties of the rare earth magnet of the present disclosure can be regarded as substantially the same as those when y is 0.

Excessively increasing the purity of raw materials of essential components entails a rise in the production cost, and therefore the value of y may be 0.01 or more, 0.02 or more, 0.03 or more, 0.04 or more, or 0.05 or more. On the other hand, the value of y is preferably lower as long as a rise in the production cost is not caused, and the value may be 0.09 or less, 0.08 or less, 0.07 or less, or 0.06 or less.

When the total content p of Nd, Ce, La and R¹ is 5.0 at% or more, the main phase represented by (Nd, Ce, La)₂Fe₁₄B is not difficult to be formed. From the viewpoint that the main phase represented by (Nd, Ce, La)₂Fe₁₄B is readily formed, p may be 7.0 at% or more, 9.0 at% or more, 11.0 at% or more, or 13.0 at% or more. On the other hand, when p is 20.0 at% or less, the existence ratio (volume ratio) of the grain boundary phase does not become excessive. From the viewpoint that the exsistence ratio of the grain boundary phase does not become excessive, the total content may be 19.0 at% or less, 18.0 at% or less, or 17.0 at% or less.

### <B>

B affects the content of the main phase and the content of the Fe-containing magnetic phase in the grain boundary phase. If the content of B is too small, the main phase represented by (Nd, Ce, La)₂Fe₁₄B is difficult to be formed. When the content r of B is 4.0 at% or more, it is unlikely that the main phase represented by (Nd, Ce, La)₂Fe₁₄B is difficult to be formed. From this viewpoint, r may be 4.5 at% or more, 5.0 at% or more, or 5.5 at% or more. On the other hand, if the content r of B is excessive, an Fe-containing magnetic phase such as RFe₄B₄ phase is readily formed in the grain boundary phase. When r is 6.5 at% or less, an α-Fe phase is less
likely to be formed in a large amount. From this viewpoint, r may be 6.3 at% or less, or 6.0 at% or less.

### <Co>

Co can substitute for iron in the main phase, grain boundary phase and intermediate phase. When Fe is referred to in the present description, part of Fe can be replaced by Co. For example, part of Fe of the (Nd, Ce, La)₂Fe₁₄B phase is replaced by Co to form the (Nd, Ce, La)₂(Fe, Co)₁₄B phase. In addition, the Fe-containing magnetic phase (e.g., R₂Fe₁₇ phase) in the grain boundary phase allows part of Fe thereof to be replaced by Co and becomes a magnetic phase (e.g., R₂(Fe, Co)₁₇ phase).

In this way, part of Fe is replaced by Co, and the Curie point in each phase is thereby enhanced. In the case of preferring not to enhance the Curie point, Co may not be contained. It is not essential to contain Co. When the content q of Co is 0.5 at% or more, enhancement of the Curie point is substantially recognized. From the viewpoint of enhancing the Curie point, the content may be 1.0 at% or more, 2.0 at% or more, 3.0 at% or more, or 4.0 at% or more. On the other hand, Co is expensive, and therefore, in economic terms, the content q of Co may be 8.0 at% or less, 7.0 at% or less, or 0.6 at% or less.

### <M¹>

M¹ may be contained within the range not compromising the properties of the rare earth magnet of the present disclosure. M¹ may contain an unavoidable impurity element. The unavoidable impurity element indicates an impurity element that is unavoidably contained or causes a significant rise in the production cost for avoiding its inclusion, such as impurity element contained in raw materials of the rare earth magnet or impurity element mixed in the production step. The impurity element, etc. mixed in the production step encompass an element incorporated due to manufacturing reasons within a range not affecting the magnetic properties.

The element that can be incorporated within a range not affecting the properties of the rare earth magnet of the present disclosure includes Ga, Al, Cu, Au, Ag, Zn, In, and Mn.

Ga, Al, Zn, In, Au, Ag and Cu decrease the melting point of the grain boundary phase present inside of a ribbon, etc. obtained, for example, by a liquid quenching method. For this reason, in the case of obtaining a molded body from a plurality of ribbons and/or obtaining a compressed body from the molded body, such elements may be incorporated so as to, for example, enhance the mold life but are not essential. When the content of M¹ is not more than the upper limit, the elements exert substantially no effect on the magnetic properties. In view of magnetic properties, these elements may be regarded as an unavoidable impurity element.

Mn contributes to the stabilization of (Nd, Ce, La)₂Fe₁₄B phase by replacing part of Fe in the (Nd, Ce, La)₂Fe₁₄B phase.

When the content s of M¹ is 2.0 at% or less, the magnetic properties of the present disclosure are not compromised. From this viewpoint, the content s of M¹ may be 1.5 at% or less, 1.0 at% or less, or 0.5 at% or less.

In the case of not containing Ga, Al, Cu, Au, Ag, Zn, In, and Mn as M¹, since it is impossible not to contain an unavoidable impurity element at all, the lower limit of the content s of M¹ may be 0.05 at%, 0.1 at%, or 0.2 at%, and this poses no practical problem.

Each of the values of p, q, r and s described hereinbefore is the same as that in the case of a normal R-Fe-B-based rare earth magnet.

### <Fe>

Fe is the remainder after removing Nd, Ce, La, R¹, Co, B, and M¹ described hereinbefore, and the content (at%) of Fe is represented by (100-p-q-r-s). When p, q, r and s are in the ranges above, a main phase and a grain boundary phase are obtained. In addition, when the rare earth magnet having a main phase and a grain boundary phase is used as a precursor and a modifier is sufficiently infiltrated into the precursor, an intermediate phase is obtained. The main phase, grain boundary phase and intermediate phase are described below.

### <Main Phase, Grain Boundary Phase, and Intermediate Phase>

Fig. 2 is a diagram schematically illustrating one embodiment of the texture of the rare earth magnet according to the present disclosure. Fig. 3 is a diagram illustrating another embodiment of the texture of the rare earth magnet according to the present disclosure.

In the embodiment illustrated in Fig. 2, the rare earth magnet 100 of the present disclosure has a main phase 10 and a grain boundary phase 20. In the embodiment illustrated in Fig. 3, the rare earth magnet 100 of the present disclosure further has an intermediate phase 30, in addition to a main phase 10 and a grain boundary phase 20.

The embodiment illustrated in Fig. 2 is recognized when a modifier is not infiltrated or a very small amount of a modifier is infiltrated. The rare earth magnet 100 of the embodiment illustrated in Fig. 2 is used as a rare earth magnet precursor into which a modifier is infiltrated. The embodiment illustrated in Fig. 3 is recognized when a sufficient amount of a modifier is infiltrated.

The rare earth magnet 100 may have a phase (not shown) other than the main phase 10, the grain bounder phase 20, and the intermediate phase 30. The phase other than the main phase 10, the grain bounder phase 20, and the intermediate phase 30 includes an oxide, a nitride, an intermetallic compound, etc.

The properties of the rare earth magnet 100 are exerted mainly by the main phase 10, the grain boundary phase 20, and the intermediate phase 30. Most of the phases other than the main phase 10, the grain boundary phase 20, and the intermediate phase 30 are an impurity. Accordingly, the total content of the main phase 10, the grain boundary phase 20, and the intermediate phase 30 is preferably 95 vol% or more, more preferably 97 vol% or more, still more preferably 99 vol% or more, relative to the rare earth magnet 100.

The main phase 10 is nanocrystallized. Being nanocrystallized means that the average grain size of the main phase 10 is from 1 to 1,000 nm. The average grain size may be 10 nm or more, 50 nm or more, or 100 nm or more, and may be 900 nm or less, 700 nm or less, 500 nm or less, or 300 nm or less.

The "average grain size" indicates an average value of longitudinal lengths t of main phases 10, for example, illustrated in Fig. 2. For example, a given region is specified in a scanning electron microscope image or a transmission electron microscope image of the rare earth magnet 100, and the average value of respective lengths t of main phases 10 present in the given region is calculated and defined as the "average grain size". In the case where the crosssectional shape of the main phase 10 is elliptic, t is denoted as the length of the long axis, and in the case where the cross-section of the main phase is quadrilateral, t is denoted as the length of a longer diagonal. In the case of the embodiment illustrated in Fig. 3, t is set including the intermediate phase 30, because, as described later, the intermediate phase 30 is derived from the main phase 10.

When the rare earth magnet 100 illustrated in Fig. 2 is used as a rare earth magnet precursor (hereinafter, sometimes referred to as "precursor 100") and a modifier is infiltrated thereinto, the modifier reaches the interface of the main phase 10 and the grain boundary 20 via the grain bounder phase 20. Then, R² in the modifier infiltrates the inside of the main phase 10 from the grain boundary phase 20 and, as illustrated in Fig. 3, an intermediate phase 30 is formed.

The grain boundary phase 20 is present around the main phase 10. The intermediate phase 30 is sandwiched between the main phase 10 and the grain boundary phase 20. Formation of the intermediate phase 30 is described by referring to the composition of the modifier.

### <R², R³, and M²>

The modifier contains an alloy having a composition represented by R²_{z}R³_{w}M²_{1-z-w}. On the other hand, the precursor 100 has a composition represented by (Ndₓ(Ce, La)_{(1-x-y})R¹_{y})ₚFe_{(100-p-q-r-s)}Co_{q}BᵣM¹ₛ.

R² is one or more members selected from Pr, Nd, Pm, Sm, Eu and Gd, and R³ is one or more members selected from rare earth elements other than R². In addition, M² represents an alloy element for decreasing the melting point of R²_{z}R³_{w}M²_{1-z-w} to be lower than the melting point of R² by alloying with R² and R³, and an unavoidable impurity element.

The precursor 100 contains mainly Nd, Ce and La as the rare earth element. On the other hand, the alloy in the modifier contains mainly R² that is one or more members selected from Pr, Nd, Pm, Sm, Eu, and Gd.

R² of the modifier differs in the kind of one or more rare earth elements from Nd, Ce and La of the precursor 100, and therefore, although not bound by theory, R² infiltrates into the main phase 10 and forms the intermediate phase 30. Accordingly, the concentration of R² is higher in the intermediate phase 30 than in the main phase 10. Although not bound by theory, the reason for infiltration of R² into the main phase 10 is considered as follows.

At the time of infiltrating the modifier into the precursor 100, when the alloy in the modifier contains mainly the same rare earth element of the main phase 10, the rare earth element in the modifier is not easily infiltrated into the main phase 10. For example, at the time of infiltrating a modifier containing an Nd-Cu alloy into the Nd-Fe-B-based rare earth magnet precursor, Nd in the modifier is likely to stay in the grain boundary phase 20 and hardly infiltrates into the main phase (Nd₂Fe₁₄B phase).

On the other hand, when the alloy in the modifier contains mainly a rare earth element different from the main phase 10, the rare earth element in the modifier readily infiltrates into the main phase 10. For example, at the time of infiltrating a modifier containing an Nd-Cu alloy into the (Nd, Ce, La)-Fe-B-based rare earth magnet, Nd in the modifier readily infiltrates into the main phase 10 due to the presence of Ce and La. From the viewpoint of enhancing the saturation magnetization and anisotropic magnetic field of the intermediate phase 30 in a balanced manner, R² is preferably Nd.

The composition of the alloy in the modifier is represented by R²_{z}R³_{w}M²_{1-z-w}. R³ is one or more members selected from rare earth elements other than R². The rare earth element contained in the alloy in the modifier is R², and it is difficult not to contain the rare earth element R³ other than R² at all. However, when the value of the content ratio w of R³ is from 0 to 0.1, the properties as the modifier can be regarded as substantially the same as those when w is 0.

The value of w is ideally close to 0, but the value of w may be 0.01 or more, 0.02 or more, 0.03 or more, 0.04 or more, or 0.05 or more. On the other hand, the value of w is preferably lower as long as a rise in the production cost is not caused, and the value may be 0.09 or less, 0.08 or less, 0.07 or less, or 0.06 or less.

In the formula: (Ndₓ(Ce, La)_{(1-x-y)}R¹_{y})ₚFe_{(100-p-q-r-s)}Co_{q}BᵣM¹ₛ·(R²_{z}R³_{w}M²_{1-z-w})ₜ of the overall composition, the value of t corresponds to the infiltration amount (at%) of the alloy from the modifier relative to the precursor 100. The concentration of R² in the intermediate phase 30 and the thickness of the intermediate phase 30 are changed according to the value of t.

In Fig. 3, when the concentration of R² is higher by 1.5 times or more in the intermediate phase 30 than in the main phase 10, the magnetic isolation can be clearly recognized. On the other hand, even when the concentration of R² is higher by 8.0 times in the intermediate phase 30 than in the main phase 10, the effect of magnetic isolation is not saturated. Accordingly, the concentration of R² is preferably higher by 1.5 to 8.0 times in the intermediate phase 30 than in the main phase 10. The concentration of R² may be higher by 1.5 to 5.0 times, or by 1.5 to 3.0 times.

In order to clearly recognize the function as the intermediate phase 30, the thickness of the intermediate phase 30 is preferably 2 nm or more, more preferably 10 nm or more, still more preferably 20 nm or more. On the other hand, the thickness of the intermediate phase 30 depends on the infiltration amount of the modifier. The modifier contains M² not contributing to magnetization, and therefore, if the infiltration amount of M² is too large, the volume fraction of the grain boundary phase is increased, and magnetization of the rare earth magnet 100 decreases. From this viewpoint, the thickness of the intermediate phase 30 is preferably 100 nm or less, more preferably 70 nm or less, still more preferably 40 nm or less.

### «Production Method»

The production method of the rare earth magnet of the present disclosure is described below.

### <Preparation of Molten Metal>

A molten metal having a composition represented by the formula: (Ndₓ(Ce, La)_{(1-x-y)}R¹_{y})ₚFe_{(100-p-q-r-s)}Co_{q}BᵣM¹ₛ and containing La in an amount of 1/9 to 3 times by molar ratio relative to Ce is prepared. Alternatively, a molten metal containing La in an amount of 1/9 to 2 times by molar ratio relative to Ce may be prepared. Descriptions regarding Nd, Ce, La, R¹, Fe, Co, B, and M¹ and regarding x, y, p, q, r, and s are the same as those in the rare earth magnet. Incidentally, in the case where a specific component is consumed during preparation of the molten metal or in the subsequent step, the component may be blended by taking into account the consumption.

The method for preparing a molten metal is not limited and includes, for example, induction heating of raw materials by using high frequency current. The preparation of a molten metal is preferably performed in an inert gas atmosphere so as to prevent oxidation of the raw materials during melting or the molten metal during storage.

### <Preparation of Ribbon>

The molten metal above is quenched to obtain a ribbon. As long as the main phase in the ribbon can be nanocrystallized, the quenching method is not particularly limited and includes, for example, a liquid quenching method. In order to nanocrystallize the main phase in the ribbon, the molten metal-cooling rate may be, typically, 1×10² K/sec or more, 1×10³ K/sec or more, or 1×10⁴ K/sec or more, and may be 1×10⁷ K/sec or less, 1×10⁶ K/sec or less, or 1×10⁵ K/sec or less.

As to the conditions in the liquid quenching method, for example, a molten metal is discharged toward a copper-made single roll in an inert gas atmosphere under reduced pressure of 50 kPa or less to obtain a ribbon, but the conditions are not limited thereto.

The molten metal discharging temperature may be, typically, 1,300°C or more, 1,350°C or more, or 1,400°C or more, and may be 1,600°C or less, 1,550°C or less, or 1500°C or less.

The peripheral velocity of the single roll may be, typically, 20 m/s or more, 24 m/s or more, or 28 m/s or more, and may be 40 m/s or less, 36 m/s or less, or 32 m/s or less.

### <Preparation of Molded Body>

The ribbon obtained by liquid quenching is compressed by hot working to obtain a molded body. The molded body is obtained from a plurality of ribbons. The method for compression is not particularly limited but includes, for example, a method where ribbons are charged into a die and hot-pressed. Before hot pressing, the ribbon may be pulverized to 10 µm or less. The temperature at the time of hot pressing may be a temperature at which a molded body is obtained, but may also be a temperature at which part of the grain boundary phase in the ribbon melts, that is, the ribbon may be liquid phase sintered. The atmosphere during hot pressing is preferably an inert gas atmosphere so as to prevent oxidation of the ribbon and molded body. In addition, as for the hot pressing, a powder obtained by pulverizing the ribbon may be compacted to obtain a compact, and the compact may then be sintered (including liquid phase sintering).

The pressure at the time of hot pressing may be, typically, 200 MPa or more, 300 MPa or more, or 350 MPa or more, and may be 600 MPa or less, 500 MPa or less, or 450 MPa or less.

The temperature at the time of hot pressing may be, typically, 550°C or more, 600°C or more, or 630°C or more, and may be 750°C or less, 700°C or less, or 670°C or less.

The pressing time at the time of hot pressing may be, typically, 5 seconds or more, 20 seconds or more, or 40 seconds or more, an may be 120 seconds or less, 100 seconds or less, or 80 seconds or less.

### <Preparation of Compressed Body>

The above-described molded body is further plastically worked by hot working to obtain a compressed body (plastically deformed body). The method for hot-plastic working (hereinafter, sometimes simply referred to as "plastic working") is not particularly limited as long as a compressed body having anisotropy is obtained. The method includes, for example, a method where the molded body is charged into a cemented carbide-made mold and plastically worked at a reduction ratio of 10 to 75%. The method for plastic working includes upsetting, backward extrusion, etc. The reduction ratio may be set to obtain desired anisotropy. The temperature at the time of plastic working may be set such that the compressed body is not broken and the crystal grain in the compressed body is not coarsened.

The reduction ratio at the time of plastic working may be, typically, 10% or more, 30% or more, 50% or more, or 60% or more, and may be 75% or less, 70% or less, or 65% or less.

The temperature at the time of plastic working may be 650°C or more, 700°C or more, or 720°C or more, and may be 850°C or less, 800°C or less, or 770°C or less.

The strain rate at the time of plastic working may be 0.001/s or more, 0.01/s or more, 0.1/s or more, or 1.0/s or more, and may be 10.0/s or less, 5.0/s or less, or 3.0/s or less.

Although not bound by theory, it is considered that the followings are generated inside the molded body during plastic working. The molded body has a main phase 10 and a grain boundary phase 20 present around the main phase 10 (see, Fig. 2). When the molded body is plastically worked, the main phase 10 is deformed. At this time, in at least part of the main phase 10, a portion allowing for direct contact between main phases 10 is likely to be produced due to the deformation. This contact part may work out to origin of the grain growth of the main phase 10. If the strain rate at the time of plastic working is low, the main phase 10 readily undergoes grain growth from the contact part as a starting point. The plastic working is performed as hot working, and therefore, when the strain rate is low, this means that the contact part above is subjected to a high temperature over a long period of time. Consequently, atomic diffusion occurs via the contact part, and the main phase 10 undergoes grain growth. On the other hand, in the initial stage of plastic working, Ce and La, particularly, La, are expelled to the grain boundary phase 20 from the main phase 10. At the time of deformation of the main phase 10 resulting from expelling of Ce and La, Ce and La enter between main phases 10, and formation of the contact part above is suppressed. In addition, due to expelling of Ce and La, the melting point of the grain boundary phase 20 lowers. The plastic working is performed at a temperature allowing at least one grain boundary phase 20 to melt. Lowering of the melting point of the grain boundary phase 20 causes reduction in the viscosity of the melt of the grain boundary phase 20 during plastic working. As a result, the main phase 10 undergoing deformation is readily rotated in the melt to facilitate orientation of the main phase 10 in a specific direction. For this reason, when the strain rate is low, typically, even when the strain rate is 0.001/s or more and less than 0.01/s, the grain growth of the main phase 10 is restricted to suppress reduction in the coercive force and at the same time, orientation of the main phase 10 is promoted to enhance the magnetization. From this viewpoint, the strain rate may be from 0.001/s to 0.008/s, or from 0.001/s to 0.005/s.

The compressed body obtained in this way may be directly used as a rare earth magnet, or by using the compressed body as a rare earth magnet precursor, subsequent steps may be performed.

### <Preparation of Modifier>

A modifier containing an alloy having a composition represented by the formula: R²_{z}R³_{w}M²_{1-z-w} is prepared. Descriptions regarding R² and R³ and regarding w are the same as those for the rare earth magnet.

M² represents an alloy element for decreasing the melting point of R²_{z}R³_{w}M²_{1-z-w} to be lower than the melting point of R² by alloying with R² and R³, and an unavoidable impurity element. Due to this element, even when the temperature of the later-described heat treatment is not raised excessively, the alloy in the modifier can be melted. As a result, the alloy in the modifier can be infiltrated into the rare earth magnet precursor without coarsening the texture of the rare earth magnet precursor. M² may contain an unavoidable impurity element. The unavoidable impurity element indicates an impurity element that is unavoidably contained or causes a significant rise in the production cost for avoiding its inclusion, such as impurity element contained in raw materials.

As M², one or more members selected from Cu, Al, and Co, and an unavoidable element are preferred, because Cu, Al, and Co have little adverse effect on the magnetic properties, etc. of the rare earth magnet.

The alloy having a composition represented by the formula: R²_{z}R³_{w}M²_{1-z-w} includes an Nd-Cu alloy, a Pr-Cu alloy, an Nd-Pr-Cu alloy, an Nd-Al alloy, a Pr-Al alloy, an Nd-Pr-Al alloy, an Nd-Co alloy, a Pr-Co alloy, and an Nd-Pr-Co alloy.

The content ratio z of R² is described. When z is 0.50 or more, the content of R² in the alloy is large, and therefore R² is easily infiltrated into the main phase 10 and the intermediate phase 30. From this viewpoint, z is preferably 0.55 or more, more preferably 0.60 or more. On the other hand, when z is 0.80 or less, the melting point of the alloy in the modifier appropriately lowers and in turn, the temperature of the later-described heat treatment is made appropriate. As a result, the texture of the rare earth magnet precursor can be prevented from coarsening. From the viewpoint of making the melting point of the alloy appropriate, z is preferably 0.75 or less, more preferably 0.70 or less. When R² is two or more elements, z is the total thereof. The same applies to M².

The production method of the modifier is not particularly limited. The production method of the modifier includes a casting method, a liquid quenching method, etc. From the viewpoint that the alloy composition less varies depending on the region of the modifier and the content of an impurity such as oxide is small, a liquid quenching method is preferred.

The infiltration amount of the alloy in the modifier is denoted by t (at%) in the formula of the overall composition. When t is 0.05 at% or more, the effect due to infiltration of the modifier is seen, for example, on the enhancement of magnetic properties. In order to clearly recognize the intermediate phase 30 as illustrated in Fig. 3, t is preferably 0.1 at% or more, more preferably 1.0 at% or more, still more preferably 1.5 at% or more. On the other hand, the modifier contains M², and therefore, if the infiltration amount of the modifier is excessive, the magnetization of the rare earth magnet after infiltration of the modifier decreases. When t is 10.0 at% or less, the decrease of magnetization poses no problem in practice. From this viewpoint, t is preferably 9.0 at% or less, more preferably 8.0 at% or less, still more preferably 7.0 at% or less.

### <Preparation of Contact Body>

The rare earth magnet precursor and the modifier are contacted with each other to obtain a contact body. The rare earth magnet precursor is the above-described compressed body. At this time, at least one surface of the rare earth magnet precursor and at least one surface of the modifier are put into contact with each other.

### <Heat Treatment>

The contact body above is heat-treated to infiltrate the melt of the modifier into the inside of the rare earth magnet precursor. The melt of the modifier thereby reaches the surface part of the main phase via the grain boundary phase of the rare earth magnet precursor, and R² in the modifier is infiltrated into the main phase to form an intermediate phase.

The heat treatment temperature is not particularly limited as long as the modifier is melted and the melt of the modifier can be infiltrated into the main phase of the rare earth magnet precursor.

As the heat treatment temperature is higher, the melt of the modifier, particularly, R², is more easily infiltrated into the main phase of the rare earth magnet precursor. From this viewpoint, the heat treatment temperature is preferably 580°C or more, more preferably 600°C or more, still more preferably 620°C or more. On the other hand, as the heat treatment temperature is lower, the texture of the rare earth magnet precursor, particularly, the main phase, is more likely to be restricted from coarsening. From this viewpoint, the heat treatment temperature is preferably 800°C or less, more preferably 775°C or less, still more preferably 725°C or less.

The heat treatment atmosphere is not particularly limited, but from the viewpoint of preventing oxidation of the rare earth magnet precursor and the modifier, an inter gas atmosphere is preferred.

### [Examples]

The rare earth magnet of the present disclosure and the production method thereof are described more specifically below by referring to Examples. Incidentally, the rare earth magnet of the present disclosure and the production method thereof are not limited to the conditions employed in the following Examples.

### <Preparation of Samples of Examples 1 to 26>

First, a rare earth magnet precursor is prepared. A molten alloy having a composition represented by R_{13.11}Fe_{80.43}Cu_{0.10}B_{5.99}Ga_{0.37} was liquid-quenched by a single roll method to obtain a ribbon. R is as in Table 1-1 later. As for the conditions of liquid quenching, the molten alloy temperature (discharge temperature) was 1,420°C, and the peripheral velocity of the roll was 30 m/s. At this time, the cooling rate of the molten alloy was 10⁶ K/sec. The liquid quenching was performed in an argon gas reduced-pressure atmosphere. It was confirmed by transmission electron microscope (TEM) observation that the ribbon is nanocrystallized.

The ribbon was roughly pulverized into a powder, and the powder was charged into die, pressurized and heated to obtain a molded body. As for the pressurizing and heating conditions, the applied pressure was 400 MPa, the heating temperature was 650°C, and the holding time for pressurization and heating was 60 seconds.

The molded body was subjected to hot upsetting (hot-plastic working) to obtain a compressed body (plastically deformed body). In the hot-plastic working, a sample of 15 mm in height was compressed to 4.5 mm. As for the hot upsetting conditions, the working temperature was 780°C, the strain rate was 0.01/s, and the reduction ratio was 70%. It was confirmed by scanning electron microscope (SEM) that the compressed body has oriented nanocrystals. This compressed body was used as a rare earth magnet precursor.

An Nd₇₀Cu₃₀ alloy was prepared as the modifier. Nd powder and Cu powder, manufactured by Kojundo Chemical Lab. Co., Ltd., were weighed, arc-melted, and liquid-quenched to obtain a ribbon.

The rare earth magnet precursor and the modifier were put into contact with each other and heat-treated in a heating furnace. The amount of the modifier was 1.59 at%, 3.72 at%, and 5.32 at%, relative to the rare earth magnet precursor (see, Table 1-1). As for the heat treatment conditions, the heat treatment temperature was 625°C, and the heat treatment time was 165 minutes.

### <Preparation of Sample of Comparative Example 1>

The sample was prepared in the same manner as in Examples 1 to 26 other than the composition of the alloy for preparing the rare earth magnet precursor was Nd_{13.11}Fe_{80.43}Cu_{0.10}B_{5.99}Ga_{0.37} and the modifier was not infiltrated into the rare earth magnet precursor.

### <Preparation of Samples of Examples 27 to 32>

The samples were prepared in the same manner as in Examples 1 to 26 except that R of the rare earth magnet precursor was changed as in Table 1-3.

### <Preparation of Samples of Examples 33 to 36>

The samples were prepared in the same manner as in Examples 1 to 26 other than R of the rare earth magnet precursor was changed as in Table 1-3 and the modifier was not infiltrated into the rare earth magnet precursor.

### <Preparation of Samples of Examples 37 and 38>

The samples were prepared in the same manner as in Examples 1 to 26 other than the composition of the alloy for preparing the rare earth magnet precursor was R_{13.11}Fe_{80.80}Cu_{0.10}B_{5.99} and R of the rare earth magnet precursor was changed as in Table 1-3.

### <Preparation of Sample of Example 39>

The sample was prepared in the same manner as in Example 6 other than the strain rate at the time of hot upsetting of the molded body was changed to 0.001/s.

### <Preparation of Sample of Example 40>

The sample was prepared in the same manner as in Example 12 except that the strain rate at the time of hot upsetting of the molded body was changed to 0.001/s.

### <Preparation of Sample of Comparative Example 2>

The sample was prepared in the same manner as in Examples 1 to 26 other than the composition of the alloy for manufacturing the rare earth magnet precursor was Nd_{13.11}Fe_{80.43}C_{U0.10}B_{5.99}Ga_{0.37}.

### <Preparation of Samples of Comparative Examples 3 to 7>

The samples were prepared in the same manner as in Examples 1 to 26 other than R of the rare earth magnet precursor was changed as in Table 1-3.

### <Preparation of Samples of Comparative Examples 8>

The sample of Comparative Example 8 was prepared in the same manner as in Comparative Example 1 other than R of the rare earth magnet precursor was changed as in Table 1-3.

### <Preparation of Samples of Comparative Examples 9>

The sample of Comparative Example 9 was prepared in the same manner as in Comparative Example 2 other than R of the rare earth magnet precursor was changed as in Table 1-3 and the infiltrating amount of the modifier was 3.72 at% relative to the rare earth magnet precursor. The sample of Comparative Example 9 is the same as the sample in which the modifier of 3.72 at% is infiltrated into Sample of Comparative Example 8.

### <Preparation of Samples of Comparative Examples 10>

The sample of Comparative Example 10 was prepared in the same manner as in Comparative Example 1 other than R of the rare earth magnet precursor was changed as in Table 1-3.

### <Preparation of Samples of Comparative Examples 11>

The sample of Comparative Example 11 was prepared in the same manner as in Comparative Example 2 other than R of the rare earth magnet precursor was changed as in Table 1-3 and the infiltrating amount of the modifier was 3.72 at% relative to the rare earth magnet precursor. The sample of Comparative Example 11 is the same as the sample in which the modifier of 3.72 at% is infiltrated into Sample of Comparative Example 10.

### <Preparation of Samples of Comparative Examples 12>

The sample of Comparative Example 12 was prepared in the same manner as in Comparative Example 2 other than R of the rare earth magnet precursor was changed as in Table 1-3 and the infiltrating amount of the modifier was 3.72 at% relative to the rare earth magnet precursor.

### <Evaluation>

With respect to the samples of Examples 1 to 40 and Comparative Examples 1 to 12, the coercive force and residual magnetization were measured. In the measurement, a pulse excitation-type magnetic properties measuring apparatus (maximum applied magnetic field: 15T) manufactured by Toei Industry Co., Ltd. was used. Both the coercive force and the residual magnetization were measured at 23°C, 100°C, 140°C and 160°C.

The results are shown in Tables 1-1 to 1-4 and Tables 2-1 and 2-2. In Tables 1-1 and Table 1-3, the composition of each sample is shown together. As for the coercive force and the residual magnetization, the gradient ΔHc from 23 to 160°C and the gradient ΔBr from 23 to 160°C are shown together, respectively. In Table 2-1, the conditions in hot upsetting and the average grain size are shown together. Here, the average grain size means the average grain size t of a crystal grain composed of a main phase 10 and an intermediate phase 30 (see, Fig. 3). Fig. 4 is a graph illustrating the relationship between the temperature and the cohesive force with respect to the samples of Example 15 and Comparative Example 1. Fig. 5 is a diagram illustrating the relationship between the temperature and the residual magnetization with respect to the samples of Example 15 and Comparative Example 1.

With respect to the samples of Examples 6, 12, 17, 39 and 40, the texture was observed using a scanning transmission electron microscope (STEM), and the component analysis (EDX analysis) was performed.

Figs. 6 to 26 illustrate the evaluation results. Of these, Figs. 6 to 14 are evaluation results regarding Examples and Comparative Examples shown in Tables 1-1 to 1-4, and Figs. 15 to 26 are the evaluation results regarding Examples shown in Tables 2-1 and 2-2.

Fig. 6 is a diagram illustrating the positions for texture observation and composition analysis with respect to the sample of Example 6. Fig. 7 is a diagram illustrating the results of texture observation and composition analysis with respect to the sample of Example 6 (first visual field). Fig. 8 is a diagram illustrating the results of texture observation and composition analysis with respect to the sample of Example 6 (second visual field). Fig. 9 is a diagram illustrating the positions for texture observation and composition analysis with respect to the sample of Example 12. Fig. 10 is a diagram illustrating the results of texture observation and composition analysis with respect to the sample of Example 12 (first visual field). Fig. 11 is a diagram illustrating the results of texture observation and composition analysis with respect to the sample of Example 12 (second visual field). Fig. 12 is a diagram illustrating the positions for texture observation and composition analysis with respect to the sample of Example 17. Fig. 13 is a diagram illustrating the results of texture observation and composition analysis with respect to the sample of Example 17 (first visual field). Fig. 14 is a diagram illustrating the results of texture observation and composition analysis with respect to the sample of Example 17 (second visual field).

Fig. 15 is a diagram illustrating one example of the grain size t of a crystal grain with respect to the sample of Example 39. Fig. 16 is a diagram illustrating one example of the grain size t of a crystal grain with respect to the sample of Example 40. Fig. 17 is a diagram illustrating one example of the grain size t of a crystal grain with respect to the sample of Example 6. Fig. 18 is a diagram illustrating one example of the grain size t of a crystal grain with respect to the sample of Example 12. In each of Figs. 15 to 18, the average grain size of Table 2 is an average of respective grain sizes t of crystal grains included in the visual field.

Fig. 19 is a diagram illustrating the results of texture observation and the positions for composition analysis with respect to the sample of Example 39. Fig. 20 is a diagram illustrating the results of composition analysis at a position indicated by a white line in Fig. 19. Fig. 21 is a diagram illustrating the results of texture observation and the positions for composition analysis with respect to the sample of Example 40. Fig. 22 is a diagram illustrating the results of composition analysis at a position indicated by a white line in Fig. 21. Fig. 23 is a diagram illustrating the results of texture observation and the positions for composition analysis with respect to the sample of Example 6. Fig. 24 is a diagram illustrating the results of composition analysis at a position indicated by a white line in Fig. 23. Fig. 25 is a diagram illustrating the results of texture observation and the positions for composition analysis with respect to the sample of Example 12. Fig. 26 is a diagram illustrating the results of composition analysis at a position indicated by a white line in Fig. 25. Furthermore, with respect to Examples 39, 40, 6 and 12, the peak concentrations of La and Ce in the grain boundary phase and the total peak concentration thereof are determined from Figs. 20, 22, 24 and 26, and the results are shown in Table 3.

[Table 1-1]

**Table 1-1**

| | Composition of Rare Earth Magnet Precursor (at%) | | | | | | | Modifier | | | Ratio of Rare Earths | | | |
|---|---|---|---|---|---|---|---|---|---|---|---|---|---|---|
| | | | | | | | | Composition Ratio | | Infiltration Amount (at%) | Percentage | | | Ratio |
| | Nd | Ce | La | Fe | B | Ga | Cu | Nd | Cu | | Nd | Ce | La | La/Ce |
| Example 1 | 6.555 | 5.8995 | 0.6555 | 80.43 | 5.99 | 0.37 | 0.1 | 0.7 | 0.3 | 1.593 | 50 | 45 | 5 | 1/9 |
| Example 2 | 6.555 | 5.8995 | 0.6555 | 80.43 | 5.99 | 0.37 | 0.1 | 0.7 | 0.3 | 3.7218 | 50 | 45 | 5 | 1/9 |
| Example 3 | 6.555 | 5.8995 | 0.6555 | 80.43 | 5.99 | 0.37 | 0.1 | 0.7 | 0.3 | 5.3184 | 50 | 45 | 5 | 1/9 |
| Example 4 | 6.555 | 3.933 | 2.622 | 80.43 | 5.99 | 0.37 | 0.1 | 0.7 | 0.3 | 1.593 | 50 | 30 | 20 | 2/3 |
| Example 5 | 6.555 | 3.933 | 2.622 | 80.43 | 5.99 | 0.37 | 0.1 | 0.7 | 0.3 | 3.7218 | 50 | 30 | 20 | 2/3 |
| Example 6 | 6.555 | 3.933 | 2.622 | 80.43 | 5.99 | 0.37 | 0.1 | 0.7 | 0.3 | 5.3184 | 50 | 30 | 20 | 2/3 |
| Example 7 | 7.866 | 4.7196 | 0.5244 | 80.43 | 5.99 | 0.37 | 0.1 | 0.7 | 0.3 | 1.593 | 60 | 36 | 4 | 1/9 |
| Example 8 | 7.866 | 4.7196 | 0.5244 | 80.43 | 5.99 | 0.37 | 0.1 | 0.7 | 0.3 | 3.7218 | 60 | 36 | 4 | 1/9 |
| Example 9 | 7.866 | 4.7196 | 0.5244 | 80.43 | 5.99 | 0.37 | 0.1 | 0.7 | 0.3 | 5.3184 | 60 | 36 | 4 | 1/9 |
| Example 10 | 7.866 | 3.1464 | 2.0976 | 80.43 | 5.99 | 0.37 | 0.1 | 0.7 | 0.3 | 1.593 | 60 | 24 | 16 | 2/3 |
| Example 11 | 7.866 | 3.1464 | 2.0976 | 80.43 | 5.99 | 0.37 | 0.1 | 0.7 | 0.3 | 3.7218 | 60 | 24 | 16 | 2/3 |
| Example 12 | 7.866 | 3.1464 | 2.0976 | 80.43 | 5.99 | 0.37 | 0.1 | 0.7 | 0.3 | 5.3184 | 60 | 24 | 16 | 2/3 |
| Example 13 | 9.177 | 3.5397 | 0.3933 | 80.43 | 5.99 | 0.37 | 0.1 | 0.7 | 0.3 | 1.593 | 70 | 27 | 3 | 1/9 |
| Example 14 | 9.177 | 3.5397 | 0.3933 | 80.43 | 5.99 | 0.37 | 0.1 | 0.7 | 0.3 | 3.7218 | 70 | 27 | 3 | 1/9 |
| Example 15 | 9.177 | 3.5397 | 0.3933 | 80.43 | 5.99 | 0.37 | 0.1 | 0.7 | 0.3 | 5.3184 | 70 | 27 | 3 | 1/9 |
| Example 16 | 9.177 | 2.9498 | 0.9833 | 80.43 | 5.99 | 0.37 | 0.1 | 0.7 | 0.3 | 3.7218 | 70 | 22.5 | 7.5 | 1/3 |
| Example 17 | 9.177 | 2.9498 | 0.9833 | 80.43 | 5.99 | 0.37 | 0.1 | 0.7 | 0.3 | 5.3184 | 70 | 22.5 | 7.5 | 1/3 |
| Example 18 | 9.177 | 2.3598 | 1.5732 | 80.43 | 5.99 | 0.37 | 0.1 | 0.7 | 0.3 | 1.593 | 70 | 18 | 12 | 1/3 |
| Example 19 | 9.177 | 2.3598 | 1.5732 | 80.43 | 5.99 | 0.37 | 0.1 | 0.7 | 0.3 | 3.7218 | 70 | 18 | 12 | 2/3 |
| Example 20 | 9.177 | 2.3598 | 1.5732 | 80.43 | 5.99 | 0.37 | 0.1 | 0.7 | 0.3 | 5.3184 | 70 | 18 | 12 | 2/3 |
| Example 21 | 5.244 | 5.8995 | 1.9665 | 80.43 | 5.99 | 0.37 | 0.1 | 0.7 | 0.3 | 1.593 | 40 | 45 | 15 | 2/3 |
| Example 22 | 5.244 | 5.8995 | 1.9665 | 80.43 | 5.99 | 0.37 | 0.1 | 0.7 | 0.3 | 3.7218 | 40 | 45 | 15 | 1/3 |
| Example 23 | 5.244 | 5.8995 | 1.9665 | 80.43 | 5.99 | 0.37 | 0.1 | 0.7 | 0.3 | 5.3184 | 40 | 45 | 15 | 1/3 |
| Example 24 | 10.488 | 1.9665 | 0.6555 | 80.43 | 5.99 | 0.37 | 0.1 | 0.7 | 0.3 | 1.593 | 80 | 15 | 5 | 1/3 |
| Example 25 | 10.488 | 1.9665 | 0.6555 | 80.43 | 5.99 | 0.37 | 0.1 | 0.7 | 0.3 | 3.7218 | 80 | 15 | 5 | 1/3 |
| Example 26 | 10.488 | 1.9665 | 0.6555 | 80.43 | 5.99 | 0.37 | 0.1 | 0.7 | 0.3 | 5.3184 | 80 | 15 | 5 | 1/3 |
| Comp. Ex. 1 | 13.11 | 0 | 0 | 80.43 | 5.99 | 0.37 | 0.1 | 0.7 | 0.3 | 0 | 100 | 0 | 0 | 0 |

[Table 1-2]

**Table 1-2**

| | Hc (kA/m) | | | | ΔHc | Br(T) | | | | ΔBr |
|---|---|---|---|---|---|---|---|---|---|---|
| | 23°C | 100°C | 140°C | 160°C | | 23°C | 100°C | 140°C | 160°C | |
| Example 1 | 814.419 | 535.629 | 399.056 | 331.710 | -3.523 | 1.078 | 0.969 | 0.891 | 0.804 | -0.001997 |
| Example 2 | 1028.451 | 664.597 | 486.864 | 394.509 | -4.627 | 1.086 | 0.972 | 0.880 | 0.808 | -0.002026 |
| Example 3 | 992.544 | 602.112 | 450.800 | 328.810 | -4.845 | 1.156 | 1.037 | 0.905 | 0.826 | -0.002408 |
| Example 4 | 624.456 | 460.678 | 351.232 | 331.162 | -2.141 | 1.071 | 0.939 | 0.809 | 0.746 | -0.002378 |
| Example 5 | 993.877 | 654.091 | 531.552 | 452.211 | -3.954 | 1.041 | 0.910 | 0.835 | 0.785 | -0.001874 |
| Example 6 | 1056.989 | 718.458 | 554.758 | 473.301 | -4.260 | 1.087 | 0.964 | 0.882 | 0.840 | -0.001803 |
| Example 7 | 1024.061 | 626.259 | 447.194 | 375.379 | -4.735 | 1.072 | 0.910 | 0.832 | 0.791 | -0.002048 |
| Example 8 | 1145.189 | 720.261 | 536.178 | 441.157 | -5.139 | 1.078 | 0.991 | 0.934 | 0.893 | -0.001350 |
| Example 9 | 1091.798 | 662.166 | 500.819 | 412.070 | -4.962 | 1.308 | 1.139 | 1.061 | 1.038 | -0.001972 |
| Example 10 | 671.026 | 461.698 | 378.515 | 288.120 | -2.795 | 1.243 | 1.147 | 1.060 | 0.945 | -0.002175 |
| Example 11 | 1123.707 | 774.906 | 599.760 | 514.147 | -4.449 | 1.088 | 0.999 | 0.933 | 0.868 | -0.001608 |
| Example 12 | 1259.810 | 828.061 | 634.413 | 537.040 | -5.276 | 1.097 | 0.964 | 0.911 | 0.826 | -0.001982 |
| Example 13 | 1015.358 | 610.109 | 454.955 | 373.106 | -4.688 | 1.320 | 1.192 | 1.082 | 1.040 | -0.002041 |
| Example 14 | 1298.931 | 814.498 | 610.030 | 503.485 | -5.806 | 1.173 | 1.091 | 1.018 | 0.930 | -0.001776 |
| Example 15 | 1250.872 | 753.659 | 555.621 | 465.461 | -5.733 | 1.327 | 1.162 | 1.039 | 0.987 | -0.002483 |
| Example 16 | 1380.781 | 932.803 | 723.162 | 609.482 | -5.630 | 1.121 | 1.027 | 0.953 | 0.950 | -0.001247 |
| Example 17 | 1559.062 | 1022.101 | 780.158 | 638.960 | -6.716 | 1.103 | 0.978 | 0.927 | 0.861 | -0.001762 |
| Example 18 | 918.613 | 612.147 | 472.674 | 427.437 | -3.585 | 1.166 | 1.019 | 0.924 | 0.913 | -0.001844 |
| Example 19 | 1252.048 | 807.128 | 628.219 | 530.611 | -5.266 | 1.285 | 1.159 | 1.047 | 0.976 | -0.002256 |
| Example 20 | 1460.435 | 933.822 | 721.123 | 608.854 | -6.216 | 1.114 | 1.026 | 0.972 | 0.896 | -0.001589 |
| Example 21 | 456.288 | 337.826 | 271.656 | 224.067 | -1.695 | 1.181 | 1.078 | 0.903 | 0.869 | -0.002275 |
| Example 22 | 893.054 | 593.880 | 459.346 | 379.221 | -3.751 | 1.116 | 0.989 | 0.915 | 0.767 | -0.002549 |
| Example 23 | 977.178 | 631.120 | 460.286 | 385.728 | -4.317 | 1.034 | 0.931 | 0.824 | 0.747 | -0.002097 |
| Example 24 | 736.254 | 489.216 | 367.931 | 344.882 | -2.857 | 0.971 | 0.900 | 0.841 | 0.757 | -0.001561 |
| Example 25 | 640.606 | 446.174 | 358.366 | 312.032 | -2.398 | 0.900 | 0.855 | 0.807 | 0.778 | -0.000894 |
| Example 26 | 956.480 | 613.323 | 476.829 | 430.730 | -3.838 | 0.885 | 0.781 | 0.715 | 0.695 | -0.001388 |
| Comp. Ex. 1 | 2111.200 | 1278.200 | 0.000 | 753.600 | -9.909 | 1.227 | | 1.061 | 1.020 | -0.001511 |

[Table 1-3]

**Table 1-3**

| | Composition of Rare Earth Magnet Precursor (at%) | | | | | | | Modifier | | | Ratio of Rare Earths | | | |
|---|---|---|---|---|---|---|---|---|---|---|---|---|---|---|
| | | | | | | | | Composition Ratio | | Infiltration Amount (at%) | Percentage | | | Ratio |
| | Nd | Ce | La | Fe | B | Ga | Cu | Nd | Cu | | Nd | Ce | La | La/Ce |
| Example 27 | 9.177 | 0.9833 | 2.9498 | 80.43 | 5.99 | 0.37 | 0.1 | 0.7 | 0.3 | 3.7218 | 70 | 7.5 | 23 | 3 |
| Example 28 | 9.177 | 0.9833 | 2.9498 | 80.43 | 5.99 | 0.37 | 0.1 | 0.7 | 0.3 | 5.3184 | 70 | 7.5 | 23 | 3 |
| Example 29 | 7.866 | 1.3110 | 3.9330 | 80.43 | 5.99 | 0.37 | 0.1 | 0.7 | 0.3 | 3.7218 | 60 | 10 | 30 | 3 |
| Example 30 | 7.866 | 1.3110 | 3.9330 | 80.43 | 5.99 | 0.37 | 0.1 | 0.7 | 0.3 | 5.3184 | 60 | 10 | 30 | 3 |
| Example 31 | 6.555 | 1.6388 | 4.9163 | 80.43 | 5.99 | 0.37 | 0.1 | 0.7 | 0.3 | 3.7218 | 50 | 12.5 | 38 | 3 |
| Example 32 | 6.555 | 1.6388 | 4.9163 | 80.43 | 5.99 | 0.37 | 0.1 | 0.7 | 0.3 | 5.3184 | 50 | 12.5 | 38 | 3 |
| Example 33 | 9.177 | 0.9833 | 2.9498 | 80.43 | 5.99 | 0.37 | 0.1 | 0 | 0 | 0 | 70 | 7.5 | 23 | 3 |
| Example 34 | 7.866 | 1.3110 | 3.9330 | 80.43 | 5.99 | 0.37 | 0.1 | 0 | 0 | 0 | 60 | 10 | 30 | 3 |
| Example 35 | 9.177 | 2.9498 | 0.9833 | 80.43 | 5.99 | 0.37 | 0.1 | 0 | 0 | 0 | 70 | 22.5 | 7.5 | 1/3 |
| Example 36 | 6.555 | 1.6388 | 4.9163 | 80.43 | 5.99 | 0.37 | 0.1 | 0 | 0 | 0 | 50 | 12.5 | 38 | 3 |
| Example 37 | 9.177 | 2.9498 | 0.9833 | 80.80 | 5.99 | 0 | 0.1 | 0.7 | 0.3 | 3.7218 | 70 | 22.5 | 7.5 | 1/3 |
| Example 38 | 9.177 | 2.9498 | 0.9833 | 80.80 | 5.99 | 0 | 0.1 | 0.7 | 0.3 | 5.3184 | 70 | 22.5 | 7.5 | 1/3 |
| Comp. Ex. 1 | 13.110 | 0 | 0 | 80.43 | 5.99 | 0.37 | 0.1 | 0.7 | 0.3 | 0 | 100 | 0 | 0 | 0 |
| Comp. Ex. 2 | 13.110 | 0 | 0 | 80.43 | 5.99 | 0.37 | 0.1 | 0.7 | 0.3 | 5.3184 | 100 | 0 | 0 | 0 |
| Comp. Ex. 3 | 9.833 | 3.2775 | 0 | 80.43 | 5.99 | 0.37 | 0.1 | 0.7 | 0.3 | 5.3184 | 75 | 25 | 0 | 0 |
| Comp. Ex. 4 | 6.555 | 6.5550 | 0 | 80.43 | 5.99 | 0.37 | 0.1 | 0.7 | 0.3 | 5.3184 | 50 | 50 | 0 | 0 |
| Comp. Ex. 5 | 3.278 | 9.8325 | 0 | 80.43 | 5.99 | 0.37 | 0.1 | 0.7 | 0.3 | 5.3184 | 25 | 75 | 0 | 0 |
| Comp. Ex. 6 | 0 | 13.1100 | 0 | 80.43 | 5.99 | 0.37 | 0.1 | 0.7 | 0.3 | 5.3184 | 0 | 100 | 0 | 0 |
| Comp. Ex. 7 | 0 | 9.8325 | 3.2775 | 80.43 | 5.99 | 0.37 | 0.1 | 0.7 | 0.3 | 5.3184 | 0 | 75 | 25 | 1/3 |
| Comp. Ex. 8 | 12.979 | 0 | 0.1311 | 80.43 | 5.99 | 0.37 | 0.1 | 0 | 0 | 0 | 99 | 0 | 1 | - |
| Comp. Ex. 9 | 12.979 | 0 | 0.1311 | 80.43 | 5.99 | 0.37 | 0.1 | 0.7 | 0.3 | 3.7218 | 99 | 0 | 1 | - |
| Comp. Ex. 10 | 12.455 | 0 | 0.6555 | 80.43 | 5.99 | 0.37 | 0.1 | 0 | 0 | 0 | 95 | 0 | 5 | - |
| Comp. Ex. 11 | 12.455 | 0 | 0.6555 | 80.43 | 5.99 | 0.37 | 0.1 | 0.7 | 0.3 | 3.7218 | 95 | 0 | 5 | - |
| Comp. Ex. 12 | 10.488 | 0 | 2.6220 | 80.43 | 5.99 | 0.37 | 0.1 | 0.7 | 0.3 | 3.7218 | 80 | 0 | 20 | - |

[Table 1-4]

**Table 1-4**

| | Hc (kA/m) | | | | ΔHc | Br (T) | | | | ΔBr |
|---|---|---|---|---|---|---|---|---|---|---|
| | 23°C | 100°C | 140°C | 160°C | | 23°C | 100°C | 140°C | 160°C | |
| Example 27 | 1209.320 | 773.416 | 610.893 | 538.765 | -4.895 | 1.140 | 1.000 | 0.963 | 0.909 | -0.001688 |
| Example 28 | 1321.902 | 874.709 | 676.984 | 587.216 | -5.363 | 1.070 | 0.990 | 0.915 | 0.845 | -0.001644 |
| Example 29 | 843.584 | 553.896 | 451.270 | 393.333 | -3.287 | 1.113 | 1.028 | 0.937 | 0.876 | -0.001726 |
| Example 30 | 1011.438 | 655.267 | 527.789 | 469.067 | -3.959 | 1.003 | 0.892 | 0.812 | 0.760 | -0.001773 |
| Example 31 | 227.909 | 174.283 | 138.376 | 120.266 | -0.786 | 1.167 | 1.007 | 0.954 | 0.885 | -0.002055 |
| Example 32 | 759.147 | 513.050 | 422.654 | 380.318 | -2.765 | 1.068 | 0.903 | 0.819 | 0.768 | -0.002194 |
| Example 33 | 309.445 | 192.002 | 157.662 | 143.394 | -1.212 | 1.188 | 0.903 | 0.833 | 0.797 | -0.002857 |
| Example 34 | 204.389 | 140.493 | 112.896 | 87.651 | -0.852 | 1.179 | 1.023 | 0.856 | 0.859 | -0.002335 |
| Example 35 | 464.050 | 300.899 | 245.706 | 226.890 | -1.731 | 1.299 | 1.141 | 1.007 | 0.948 | -0.002561 |
| Example 36 | 172.166 | 87.886 | 79.890 | 69.776 | -0.747 | 1.141 | 1.079 | 1.022 | 0.999 | -0.001037 |
| Example 37 | 924.101 | 555.778 | 407.837 | 338.923 | -4.271 | 1.312 | 1.162 | 1.021 | 0.993 | -0.002331 |
| Example 38 | 978.118 | 572.242 | 438.178 | 350.134 | -4.584 | 1.267 | 1.105 | 0.969 | 0.940 | -0.002383 |
| Comp. Ex. 1 | 2111.200 | 1278.200 | 857.905 | 753.600 | -9.909 | 1.227 | 1.132 | 1.061 | 1.020 | -0.001511 |
| Comp. Ex. 2 | 2213.500 | 1380.240 | 956.376 | 850.460 | -9.949 | 1.110 | 1.016 | 0.960 | 0.930 | -0.001314 |
| Comp. Ex. 3 | 1593.680 | 962.400 | 708.184 | 589.760 | -7.328 | 1.090 | 0.999 | 0.922 | 0.875 | -0.001569 |
| Comp. Ex. 4 | 1344.000 | 756.000 | 524.000 | 378.080 | -7.051 | 1.040 | 0.953 | 0.880 | 0.835 | -0.001497 |
| Comp. Ex. 5 | 518.160 | 353.440 | 250.400 | 196.640 | -2.347 | 0.845 | 0.614 | 0.541 | 0.432 | -0.003012 |
| Comp. Ex. 6 | 405.600 | 262.400 | 160.800 | 105.600 | -2.190 | 0.805 | 0.619 | 0.546 | 0.383 | -0.003081 |
| Comp. Ex. 7 | 405.600 | 262.400 | 160.800 | 105.600 | -2.190 | 0.851 | 0.581 | 0.544 | 0.431 | -0.003064 |
| Comp. Ex. 8 | 1076.746 | 648.603 | 489.373 | 412.541 | -4.848 | 1.347 | 1.217 | 1.117 | 1.062 | -0.002078 |
| Comp. Ex. 9 | 1745.654 | 1101.520 | 775.611 | 691.174 | -7.697 | 1.235 | 1.102 | 1.031 | 1.003 | -0.001694 |
| Comp. Ex. 10 | 1085.370 | 663.813 | 517.440 | 445.234 | -4.673 | 1.341 | 1.201 | 1.085 | 1.016 | -0.002374 |
| Comp. Ex. 11 | 1766.587 | 1114.926 | 855.344 | 707.403 | -7.731 | 1.238 | 1.127 | 1.092 | 1.026 | -0.001547 |
| Comp. Ex. 12 | 1337.739 | 845.701 | 670.085 | 578.435 | -5.542 | 1.222 | 1.057 | 0.978 | 0.931 | -0.002123 |

It could be confirmed from Tables 1-1 to 1-4 that in all of the samples of Examples 1 to 38, the absolute value of ΔHc is smaller than in Comparative Examples 1 to 4. In addition, it could be confirmed that in all of the samples of Examples 1 to 38, the absolute value of ΔBr is very small. Furthermore, it could be confirmed that in Comparative Examples 5 to 7, the decrease of magnetization at high temperatures is large. These results could verify that in the rare earth magnet of the present disclosure, reduction in the coercive force at high temperatures can be suppressed without greatly affecting the magnetization. The same could also be verified in Figs. 4 and 5. In addition, from Figs. 6 to 11, formation of an intermediate phase 30 could be confirmed.

With regard to the samples in which the modifier are infiltrated, the samples of Examples 1 to 32 and Examples 37 to 38 are compared with the samples of Comparative Examples 9, 11, and 12. Then, it could be confirmed that, with regard to rare earth elements, the absolute value of ΔHc is smaller in the samples of Examples 1 to 32 and Examples 37 to 38 that contain Nd, Ce, and La than in the samples of Comparative Examples 9, 11, and 12 that contain only Nd and La. With regard to the samples in which the modifier are not infiltrated, the same could also be confirmed between the samples of Examples 33 to 36 and the samples of Comparative Examples 8 and 10.

[Table 2-1]

**Table 2-1**

| | Composition of Rare Earth Magnet Precursor (at%) | | | | | | Modifier | | | Ratio of Rare Earths | | | | Hot Upsetting Conditions | | | Average Grain Size (µm) |
|---|---|---|---|---|---|---|---|---|---|---|---|---|---|---|---|---|---|
| | | | | | | | Composition Ratio | | Infiltration Amount (at%) | Percentage | | | Ratio | Strain Rate (/s) | Reduction Ratio (%) | Temperature (°C) | |
| | Nd | Ce | La | Fe | B | Ga Cu | Nd | Cu | | Nd | Ce | La | La/Ce | | | | |
| Example 6 | 6.555 | 3.933 | 2.622 | 80.43 | 5.99 | 0.37 | 0.7 | 0.3 | 5.3184 | 50 | 30 | 20 | 2/3 | 0.01 | 70 | 780 | 527.72 |
| Example 12 | 7.866 | 3.1464 | 2.0976 | 80.43 | 5.99 | 0.37 0.1 | 0.7 | 0.3 | 5.3184 | 60 | 24 | 16 | 2/3 | 0.01 | 70 | 780 | 579.33 |
| Example 39 | 6.555 | 3.933 | 2.622 | 80.43 | 5.99 | 0.37 0.1 | 0.7 | 0.3 | 5.3184 | 50 | 30 | 20 | 2/3 | 0.001 | 70 | 780 | 595.82 |
| Example 40 | 7.866 | 3.1464 | 2.0976 | 80.43 | 5.99 | 0.37 0.1 | 0.7 | 0.3 | 5.3184 | 60 | 24 | 16 | 2/3 | 0.001 | 70 | 780 | 638.27 |

[Table 2-2]

**Table 2-2**

| | Hc (kA/m) | | | | ΔHc | Br (T) | | | | ΔBr |
|---|---|---|---|---|---|---|---|---|---|---|
| | 23°C | 100°C | 140°C | 160°C | | 23 °C | 100°C | 140°C | 160°C | |
| Example 6 | 1056.989 | 718.458 | 554.758 | 473.301 | -4.260 | 1.087 | 0.964 | 0.882 | 0.840 | -0.001803 |
| Example 12 | 1259.810 | 828.061 | 634.413 | 537.040 | -5.276 | 1.097 | 0.964 | 0.911 | 0.826 | -0.001982 |
| Example 39 | 857.696 | 543.939 | 406.739 | 336.650 | -3.803 | 1.221 | 1.110 | 0.979 | 0.887 | -0.002436 |
| Example 40 | 1054.088 | 637.862 | 479.888 | 399.840 | -4.776 | 1.244 | 1.124 | 1.023 | 0.971 | -0.001993 |

### [Table 3]

**Table 3**

| | Example 6 | Example 12 | Example 39 | Example 40 |
|---|---|---|---|---|
| Ce (at%) | 13.85 | 11.01 | 9.46 | 9.21 |
| La (at%) | 11.52 | 5.73 | 16.19 | 16.91 |
| Ce+La (at%) | 25.37 | 16.74 | 25.65 | 26.12 |

It could be confirmed from Table 2 that even when the strain rate is low, the increase in the average grain size of a crystal grain is suppressed and consequently, the coercive force is not deteriorated. In addition, it could be confirmed that when the strain rate is low, the magnetization is enhanced. Furthermore, it could be confirmed from Table 3 that the concentrations of Ce and La, particularly La, in the grain boundary phase 20 are high when the strain rate is low, compared with the case where the strain rate is high, and the maintenance of coercive force and the enhancement of magnetization possibly have high relevance to the expelling of Ce and La to the grain boundary phase 20 from the main phase 10.

From the results above, the effects of the rare earth magnet of the present disclosure and the production method thereof could be verified.

### [Description of Numerical References]

- 10: Main phase
- 20: Grain boundary phase
- 30: Intermediate phase
- 100: Rare earth magnet (precursor)

## Claims

1. A rare earth magnet comprising:
a main phase (10), and
a grain boundary phase (20) present around the main phase (10),
wherein the overall composition is represented by the formula: (Ndₓ(Ce, La)_{(1-x-y})R¹_{y})ₚFe_{(100-p-q-r-s)}Co_{q}BᵣM¹ₛ · (R²_{z}R³_{w}M²₁-z-w)t,
wherein R¹ is one or more members selected from rare earth elements other than Nd, Ce and La, R² is one or more members selected from Pr, Nd, Pm, Sm, Eu and Gd, R³ is one or more members selected from rare earth elements other than R², M¹ represents one or more members selected from Ga, Al, Cu, Au, Ag, Zn, In and Mn, and an unavoidable impurity element, M² represents an alloy element for decreasing the melting point of R²_{z}R³_{w}M²_{1-z-w} to be lower than the melting point of R² by alloying with R² and R³, and an unavoidable impurity element,
wherein p, q, r, s, and t are, in at%,
5.0≤p≤20.0,
0≤q≤8.0,
4.0≤r≤6.5,
0≤s≤2.0, and
0≤t≤10.0, and
wherein x, y, z, and w are, by molar ratio,
0.4≤x≤0.8,
0≤y≤0.1,
0.5≤z≤0.8, and
0≤w≤0.1), and
wherein La is contained in an amount of 1/9 to 3 times by molar ratio relative to Ce, and wherein
an average grain size of the main phase (10) is from 1 to 1000 nm wherein the
average grain size of the main phase (10) is calculated in accordance with the method
defined in the description.

2. The rare earth magnet according to claim 1, wherein La is contained in an amount of 1/9 to 2 times by molar ratio relative to Ce.

3. The rare earth magnet according to claim 1 or 2,
wherein an intermediate phase (30) is further provided between the main phase (10) and the grain boundary phase (20),
wherein t is 0.1≤t≤10.0, and
wherein the concentration of R² is higher in the intermediate phase (30) than in the main phase (10).

4. The rare earth magnet according to any one of claims 1 to 3, wherein R² is Nd.

5. The rare earth magnet according to claim 3 or 4, wherein the concentration of R² is higher by 1.5 to 8.0 times in the intermediate phase (30) than in the main phase (10).

6. The rare earth magnet according to any one of claims 3 to 5, wherein the thickness of the intermediate phase (30) is from 2 to 100 nm.

7. A method for producing a rare earth magnet, comprising:
preparing a molten metal having a composition represented by the formula: (Ndₓ(Ce, La)_{(1-x-y)}R¹_{y})ₚFe_{(100-p-q-r-s)}Co_{q}BᵣM¹ₛ,
wherein R¹ is one or more members selected from rare earth elements other than Nd, Ce and La, M¹ represents one or more members selected from Ga, Al, Cu, Au, Ag, Zn, In and Mn, and an unavoidable impurity element,
wherein p, q, r, and s are, in at%,
5.0≤p≤20.0,
0≤q≤8.0,
4.0≤r≤6.5,and
0≤s≤2.0,and
wherein x and y are, by molar ratio,
0.4≤x≤0.8, and
0≤y≤0.1, and
wherein La is contained in an amount of 1/9 to 3 times by molar ratio relative to Ce, and quenching the molten metal to obtain a ribbon,
compressing a plurality of ribbons by hot working to obtain a molded body, and
compressing the molded body by hot working to obtain a compressed body, wherein an average grain size of the main phase (10) is from 1 to 1000 nm, wherein the average grain size of the main phase (10) is calculated in accordance with the method defined in the description.

8. The method according to claim 7, wherein the molten metal contains La in an amount of 1/9 to 2 times by molar ratio relative to Ce.

9. The method according to claim 7 or 8, comprising:
preparing a modifier containing an alloy represented by the formula: R²_{z}R³_{w}M²_{1-z-w},
wherein R² is one or more members selected from Pr, Nd, Pm, Sm, Eu and Gd, R³ is one or more members selected from rare earth elements other than R², M² represents an alloy element for decreasing the melting point of R²_{z}R³_{w}M²_{1-z-w} to be lower than the melting point of R² by alloying with R² and R³, and an unavoidable impurity element, and
wherein z and w are, by molar ratio, 0.5≤z≤0.8 and 0≤w≤0.1,
contacting the compressed body and the modifier with each other to obtain a contact body, and
heat-treating the contact body to infiltrate a melt of the modifier into the inside of the compressed body.

10. The method according to claim 9, wherein R² is Nd.

11. The method according to any one of claims 7 to 10,
wherein the molded body is compressed at a strain rate of 0.001/s or more and less than 0.01/s, a reduction ratio of 50 to 70%, and a temperature of 700 to 800°C to obtain a compressed body.

## Patentansprüche

1. Seltenerdmagnet, der Folgendes umfasst:
eine Hauptphase (10), und
eine Korngrenzenphase (20), die um die Hauptphase (10) herum vorhanden ist,
wobei die Gesamtzusammensetzung durch folgende Formel dargestellt wird: (Ndₓ(Ce, La)_{(1-x-y)}R¹_{y})pFe_{(100-p-q-r-s)}Co_{q}BᵣM¹ₛ•(R²_{z}R³_{w}M²_{1-z-w})ₜ,
wobei R¹ ein oder mehrere Elemente ist, die aus anderen Seltenerdelementen als Nd, Ce und La ausgewählt sind, R² ein oder mehrere Elemente ist, die aus Pr, Nd, Pm, Sm, Eu und Gd ausgewählt sind, R³ ein oder mehrere Elemente ist, die aus anderen Seltenerdelementen als R² ausgewählt sind, M¹ ein oder mehrere Elemente, die aus Ga, Al, Cu, Au, Ag, Zn, In und Mn ausgewählt sind, und ein unvermeidbares Verunreinigungselement darstellt, M² ein Legierungselement zur Herabsetzung des Schmelzpunkts von R²_{z}R³_{w}M²_{1-z-w} unter den Schmelzpunkt von R² durch Legieren mit R² und R³ sowie ein unvermeidbares Verunreinigungselement darstellt,
wobei p, q, r, s und t in at% Folgendes sind:
5,0 ≥ p ≥ 20,0,
0 ≥ q ≥ 8,0
4,0 ≥ r ≥ 6,5,
0 ≥ s ≥ 2,0 und
0 ≥ t ≥ 10,0 und
wobei x, y, z und w im molaren Verhältnis Folgendes sind:
0,4 ≥ x ≥ 0,8,
0 ≥ y ≥ 0,1,
0,5 ≥ z ≥ 0,8 und
0 ≥ w ≥ 0,1) und
wobei La in einer Menge von 1/9 bis zum 3-fachen Molverhältnis relativ zu Ce enthalten ist, und wobei eine durchschnittliche Korngröße der Hauptphase (10) von 1 bis 1000 nm beträgt, wobei die durchschnittliche Korngröße der Hauptphase (10) gemäß dem Verfahren berechnet wird, das in der Beschreibung definiert ist.

2. Seltenerdmagnet nach Anspruch 1, wobei La in einer Menge von 1/9 bis zum 2-fachen Molverhältnis relativ zu Ce enthalten ist.

3. Seltenerdmagnet nach Anspruch 1 oder 2,
wobei ferner eine Zwischenphase (30) zwischen der Hauptphase (10) und der Korngrenzenphase (20) vorgesehen ist,
wobei t 0,1 ≥ t ≥ 10,0 ist, und
wobei die Konzentration von R² in der Zwischenphase (30) höher ist als in der Hauptphase (10).

4. Seltenerdmagnet nach einem der Ansprüche 1 bis 3, wobei R²Nd ist.

5. Seltenerdmagnet nach Anspruch 3 oder 4, wobei die Konzentration von R² in der Zwischenphase (30) um das 1,5 bis 8,0-fache höher ist als in der Hauptphase (10).

6. Seltenerdmagnet nach einem der Ansprüche 3 bis 5, wobei die Dicke der Zwischenphase (30) 2 bis 100 nm beträgt.

7. Verfahren zur Herstellung eines Seltenerdmagneten, das Folgendes umfasst:
Herstellen eines geschmolzenen Metalls mit einer Zusammensetzung, die durch folgende Formel dargestellt wird: (Ndₓ(Ce, La)_{(1-x-y)}R¹_{y})ₚFe_{(100-p-q-r-s)}Co_{q}BᵣM¹s
wobei R¹ ein oder mehrere Elemente ist, die aus anderen Seltenerdelementen als Nd, Ce und La ausgewählt sind, M¹ ein oder mehrere Elemente, die aus Ga, Al, Cu, Au, Ag, Zn, In und Mn ausgewählt sind, und ein unvermeidbares Verunreinigungselement darstellt,
wobei p, q, r und s in at% Folgendes sind:
5.0 ≥ p ≥ 20.0,
0 ≥ q ≥ 8,0,
4,0 ≥ r ≥ 6,5 und
0 ≥ s ≥ 2,0 und
wobei x und y im molaren Verhältnis Folgendes sind:
0,4 ≥ x ≥ 0,8 und
0 ≥ y ≥ 0,1 und
wobei La in einer Menge von 1/9 bis zum 3-fachen Molverhältnis relativ zu Ce enthalten ist, und
Abschrecken des geschmolzenen Metalls zum Erhalt eines Bandes,
Komprimieren einer Vielzahl von Bändern durch Warmumformung, um einen Formkörper zu erhalten, und
Komprimieren des geformten Körpers durch Warmumformung, um einen komprimierten Körper zu erhalten, wobei eine durchschnittliche Korngröße der Hauptphase (10) von 1 bis 1000 nm beträgt, wobei die durchschnittliche Korngröße der Hauptphase (10) gemäß dem Verfahren berechnet wird, das in der Beschreibung definiert ist.

8. Verfahren nach Anspruch 7, wobei das geschmolzene Metall La in einer Menge von 1/9 bis zum 2-fachen Molverhältnis relativ zu Ce enthält.

9. Verfahren nach Anspruch 7 oder 8, das Folgendes umfasst:
Herstellen eines Modifikators, der eine Legierung enthält, die durch folgende Formel dargestellt wird: R²_{z}R³_{w}M²_{1-z-w},
wobei R² ein oder mehrere Elemente ist, die aus Pr, Nd, Pm, Sm, Eu und Gd ausgewählt sind, R³ ein oder mehrere Elemente ist, die aus anderen Seltenerdelementen als R² ausgewählt sind, M² ein Legierungselement zur Herabsetzung des Schmelzpunkts von R²_{z}R³_{w}M²_{1-z-w} unter den Schmelzpunkt von R² durch Legieren mit R² und R³ sowie ein unvermeidbares Verunreinigungselement darstellt, und
wobei z und w in einem Molverhältnis von 0,5 ≥ z ≥ 0,8 und 0 ≥ w ≥ 0,1 stehen,
Inkontaktbringen des komprimierten Körpers und des Modifikators miteinander, um einen Kontaktkörper zu erhalten, und
Wärmebehandeln des Kontaktkörpers, um eine Schmelze des Modifikators in das Innere des gepressten Körpers zu infiltrieren.

10. Verfahren nach Anspruch 9, wobei R² Nd ist.

11. Verfahren nach einem der Ansprüche 7 bis 10,
wobei der Formkörper mit einer Dehnungsrate von 0,001/s oder mehr und weniger als 0,01/s, einem Reduktionsverhältnis von 50 bis 70% und einer Temperatur von 700 bis 800°C komprimiert wird, um einen komprimierten Körper zu erhalten.

## Revendications

1. Aimant aux terres rares comprenant :
une phase principale (10), et
une phase intergranulaire (20) présente autour de la phase principale (10),
dans lequel la composition globale est représentée par la formule :
(Ndₓ(Ce,La)_{(1-x-y)}R¹_{y})ₚFe_{(100-p-q-r-s)}Co_{q}BᵣM¹ₛ·(R²_{z}R³_{w}M²_{1-z-w})ₜ
dans laquelle R¹ est un ou plusieurs éléments choisis parmi les éléments des terres rares autres que Nd, Ce et La, R² est un ou plusieurs éléments choisis parmi Pr, Nd, Pm, Sm, Eu et Gd, R³ est un ou plusieurs éléments choisis parmi les éléments des terres rares autres que R², M¹ représente un ou plusieurs éléments choisis parmi Ga, Al, Cu, Au, Ag, Zn, In et Mn, et un élément d'impureté inévitable, M² représente un élément d'alliage pour diminuer le point de fusion de R²_{z}R³_{w}M²_{1-z-w} pour qu'il soit inférieur au point de fusion de R² en s'alliant avec R² et R³, et un élément d'impureté inévitable,
dans laquelle p, q, r, s, et t sont, en % atomique,
5,0≤p≤20,0,
0≤q≤8,0,
4,0≤r≤6,5,
0≤s≤2,0 et
0≤t≤10,0, et
dans laquelle x, y, z et w sont, en rapport molaire,
0,4≤x≤0,8,
0≤y≤0,1,
0,5≤z≤0,8 et
0≤w≤0,1, et
dans laquelle La est contenu en une quantité de 1/9 à 3 fois en rapport molaire par rapport à Ce, et dans laquelle une granulométrie moyenne de la phase principale (10) est de 1 à 1000 nm, dans laquelle la granulométrie moyenne de la phase principale (10) est calculée selon le procédé défini dans la description.

2. Aimant aux terres rares selon la revendication 1, dans lequel La est contenu à raison de 1/9 à 2 fois en rapport molaire par rapport à Ce.

3. Aimant aux terres rares selon la revendication 1 ou 2,
dans lequel une phase intermédiaire (30) est en outre prévue entre la phase principale (10) et la phase intergranulaire (20),
dans lequel t est 0,1≤t≤10,0, et
dans lequel la concentration de R² est plus élevée dans la phase intermédiaire (30) que dans la phase principale (10).

4. Aimant aux terres rares selon l'une quelconque des revendications 1 à 3, dans lequel R² est Nd.

5. Aimant aux terres rares selon la revendication 3 ou 4, dans lequel la concentration de R² est plus élevée de 1,5 à 8,0 fois dans la phase intermédiaire (30) que dans la phase principale (10).

6. Aimant aux terres rares selon l'une quelconque des revendications 3 à 5, dans lequel l'épaisseur de la phase intermédiaire (30) est de 2 à 100 nm.

7. Procédé de production d'un aimant aux terres rares, comprenant :
la préparation d'un métal fondu ayant une composition représentée par la formule :
(Ndₓ(Ce,La)_{(1-x-y)}R¹_{y})ₚFe_{(100-p-q-r-s)}Co_{q}BᵣM¹ₛ
dans laquelle R¹ est un ou plusieurs éléments choisis parmi les éléments des terres rares autres que Nd, Ce et La, M¹ représente un ou plusieurs éléments choisis parmi Ga, Al, Cu, Au, Ag, Zn,
In et Mn, et un élément d'impureté inévitable,
dans laquelle p, q, r et s sont, en % atomique,
5,0≤p≤20,0,
0≤q≤8,0,
4,0≤r≤6,5 et
0≤s≤2,0, et
dans laquelle x et y sont, en rapport molaire,
0,4≤ x≤0,8, et
0≤y≤0,1,et
dans laquelle La est contenu en une quantité de 1/9 à 3 fois en rapport molaire par rapport à Ce, et
le trempedu métal fondu pour obtenir un ruban,
lacompressiond'une pluralité de rubans par usinage à chaud pour obtenir un corps moulé, et lacompressiondu corps moulé par usinage à chaud pour obtenir un corps comprimé, dans laquelle une granulométrie moyenne de la phase principale (10) est de 1 à 1000 nm, dans laquelle la granulométrie moyenne de la phase principale (10) est calculéeselon le procédé défini dans la description.

8. Procédé selon la revendication 7, dans lequel le métal fondu contient La en une quantité de 1/9 à 2 fois en rapport molaire par rapport à Ce.

9. Procédé selon la revendication 7 ou 8, comprenant :
la préparation d'un modificateur contenant un alliage représenté par la formule :
R²_{z}R³_{w}M²_{1-z-w},
dans laquelle R² est un ou plusieurs éléments choisis parmi Pr, Nd, Pm, Sm, Eu et Gd, R³ est un ou plusieurs éléments choisis parmi des éléments de terres rares autres que R², M² représente un élément d'alliage pour diminuer le point de fusion de R²_{z}R³_{w}M²_{1-z-w}pour qu'il soit inférieur au point de fusion de R² en s'alliant avec R² et R³, et un élément d'impureté inévitable, et
dans laquelle z et w sont, en rapport molaire, 0,5≤z≤0,8 et 0≤w≤0,1,
la mise en contact du corps comprimé et du modificateur l'un avec l'autre pour obtenir un corps de contact, et
le traitement thermique du corps de contact pour infiltrer une masse fondue du modificateur à l'intérieur du corps compressé.

10. Procédé selon la revendication 9, dans lequel R² est Nd.

11. Procédé selon l'une quelconque des revendications 7 à 10,
dans lequel le corps moulé est comprimé à une vitesse de déformation de 0,001/s ou plus et inférieure à 0,01/s, un taux de réduction de 50 à 70%, et une température de 700 à 800°C pour obtenir un corps compressé.
